# EUROPEAN PATENT SPECIFICATION

(11) **EP 4 214 346 B1**
(45) Date of publication and mention of the grant of the patent: **29.01.2025**
(21) Application number: 21789984.8
(22) Date of filing: 16.09.2021
(51) Int. Cl.: C22C 21/10, C22F 1/053

(54) **METHOD OF MAKING HIGH STRENGTH AND LOW QUENCH SENSITIVE 7XXX SERIES ALUMINUM ALLOYS**
VERFAHREN ZUR HERSTELLUNG VON HOCHFESTEN UND WENIG ABSCHRECKEMPFINDLICHEN 7XXX-ALUMINIUMLEGIERUNGEN
PROCÉDÉ DE FABRICATION D'ALLIAGES D'ALUMINIUM DE LA SÉRIE 7XXX À HAUTE RÉSISTANCE ET PEU SENSIBLES À LA TREMPE

(30) Priority: 17.09.2020 US 202062706906 P
(43) Date of publication of application: 26.07.2023
(73) Proprietor: Novelis, Inc., Atlanta, GA 30326 (US)
(72) Inventor: YUAN, Yudie, Kennesaw, Georgia 30144 (US); BHASKARAN, Ganesh, Kennesaw, Georgia 30144 (US); JANOFF, Anna E., Kennesaw, Georgia 30144 (US); WU, Cedric, Kennesaw, Georgia 30144 (US); KAMAT, Rajeev G., Kennesaw, Georgia 30144 (US); LEYVRAZ, David, Kennesaw, Georgia 30144 (US)
(74) Representative: Weickmann & Weickmann PartmbB
(86) International application number: PCT/US2021/050709
(87) International publication number: WO 2022/061011

(56) References cited:
- EP-A1- 3 521 466
- WO-A1-2019/159810
- CN-A- 107 881 444
- DE-T5- 112019 000 856
- US-A1- 2017 081 749
- "Standard Practice for Slow Strain Rate Testing to Evaluate the Susceptibility of Metallic Materials to Environmentally Assisted Cracking - G129", 10 November 2000, article ASTM STANDARDS: "Standard Practice for Slow Strain Rate Testing to Evaluate the Susceptibility of Metallic Materials to Environmentally Assisted Cracking - G129", pages: 1 - 7, XP055863249
- "Standard Test Method for Standard Test Method for Plastic Strain Ratio Plastic Strain Ratio r r for Sheet Metal for Sheet Metal - E517", 31 December 2000, article ASTM STANDARDS: "Standard Test Method for Standard Test Method for Plastic Strain Ratio Plastic Strain Ratio r r for Sheet Metal for Sheet Metal - E517", pages: 1 - 8, XP055863250

## Description

### CROSS-REFERENCE TO RELATED APPLICATIONS

This application claims the benefit of and priority to U.S. Provisional Application No. 62/706,906, filed September 17, 2020.

### FIELD

The present disclosure relates to metallurgy generally and more specifically to methods for making aluminum alloy products having improved intergranular and stress corrosion cracking resistance.

### BACKGROUND

High strength aluminum alloys are desirable for use in a variety of applications, such as the automotive and aerospace industries. Exemplary high strength aluminum alloys include 7xxx series aluminum alloys. During the processing of a 7xxx series aluminum alloy, the alloy may undergo heat treatment followed by rapid quenching to lock in solutionized alloying elements and provide for suitable intergranular and stress corrosion cracking resistance and desirable mechanical properties. If quenching does not take place on a suitable time scale, the resultant product may be susceptible to intergranular and stress corrosion cracking and/or have unsuitable mechanical properties.

The fast quench rates required for 7xxx series aluminum alloy processing leave extremely small operating windows between the hot treatment step and the quenching step. Such a small window means that a product made from a 7xxx series aluminum alloy may need to be immediately quenched after the hot processing step, leaving little to no time for other processing steps such as hot forming or transferring the hot product between locations. Fast quench rates may also be undesirable because they often employ specialized equipment and increase processing complexity.

US 2017/0081749 A1 is directed to an Al-Zn-Mg alloy sheet comprising, in mass percent, Zn in a content of 3.0% to 6.0%, Mg in a content of 2.5% to 4.5%, Cu in a content of 0.05% to 0.5%, and wherein, the Zn content [Zn] and the Mg content [Mg] satisfies [Zn] ≥ - 0.3[Mg]+4.5, grain-boundary precipitates observed with a transmission electron microscope at 60000-total magnification have an average compositional ratio of Zn to Mg of from 0.5 to 3.0 in a microstructure of the sheet subjected to a natural aging at room temperature subsequent to a solution treatment and quenching, intergranular precipitates observed with a transmission electron microscope at 60000-total magnification have an average compositional ratio of Zn to Mg of from 1.5 to 3.5 in a microstructure of the sheet further subjected to one of a two-stage artificial aging and a single-stage artificial aging after the natural aging at room temperature, wherein the two-stage artificial aging comprises a first-stage heat treatment at a temperature of from 70° C to 100° C for 2 hours or longer, and a second-stage heat treatment at a temperature of from 100° C to 170° C for 5 hours or longer, and the single-stage artificial aging comprises a heat treatment at a temperature of from 100° C to 150° C for 12 to 36 hours.

WO 2019/159810 A1 is directed to a method for the manufacture of an aluminum alloy member in which the member made from a heat-treatable aluminum alloy material is subjected to a solution heat treatment at 440 to 580°C followed by a quenching treatment in which quenching with a quenching rate of 10°C/s or more in a temperature range from the temperature of the solution heat treatment to at least 100°C is carried out and finally holding the material at a holding temperature of -196°C or higher and 40°C or lower to suppress natural ageing and afterwards performing a forming treatment characterized therein that in tensile tests, which are carried out at 20°C on a test specimen of the material prior the forming operation, the tensile strength is 465 MPa or less and the yield strength is 295 MPa or less.

EP 3 521 466 A1 is directed to a 7xxx aluminum alloy comprising 4 - 15 wt. % Zn, 0.1 - 3.5 wt. % Cu, 1.0 - 4.0 wt. % Mg, 0.05 - 0.50 wt. % Fe, 0.05 - 0.30 wt. % Si, 0.05 - 0.25 wt. % Zr, up to 0.25 wt. % Mn, up to 0.20 wt. % Cr, up to 0.15 wt. % Ti, up to 0.15 wt. % of impurities, with the remainder as Al, and optionally further comprising up to 0.20 % of one or more of Mo, Nb, Be, B, Co, Sn, Sr, V, In, Hf, Ag, Sc, and Ni and/or optionally further comprising up to 0.10 % of a rare earth element selected from the group consisting of Y, La, Ce, Pr, Nd, Pm, Sm, Eu, Gd, Tb, Dy, Ho, Er, Tm, Yb, and Lu.

### SUMMARY

The term embodiment and like terms are intended to refer broadly to all of the subject matter of this disclosure and the claims below. Statements containing these terms should be understood not to limit the subject matter described herein or to limit the meaning or scope of the claims below. Embodiments of the present disclosure covered herein are defined by the claims below, not this summary. This summary is a high-level overview of various aspects of the disclosure and introduces some of the concepts that are further described in the Detailed Description section below. This summary is not intended to identify key or essential features of the claimed subject matter, nor is it intended to be used in isolation to determine the scope of the claimed subject matter. The subject matter should be understood by reference to appropriate portions of the entire specification of this disclosure, any or all drawings and each claim.

The invention is defined in the appended claims. Described herein are rolled aluminum alloy products and methods of making aluminum alloy products having quench insensitivity and improved strength values. The methods of making aluminum alloy products include heating a rolled aluminum alloy product. The rolled aluminum alloy product includes a 7xxx series aluminum alloy product having from 4.00 wt.% to 15.00 wt.% Zn, from 0.30 wt.% to 2.50 wt.% Cu, from 1.60 wt.% to 2.60 wt.% Mg, from 0.10 wt.% to 0.25 wt.% Fe, from 0.07 wt.% to 0.15 wt.% Si, from 0.09 wt.% to 0.15 wt.% Zr, from 0.02 wt.% to 0.05 wt.% Mn, from 0.03 wt.% to 0.05 wt.% Cr, from 0.003 wt.% to 0.035 wt.% Ti, and remainder Al, with a maximum of 0.15 wt.% for the sum of all impurities, or having from 4.00 wt.% to 15.00 wt.% Zn, from 0.20 wt.% to 2.10 wt.% Cu, from 2.20 wt.% to 2.40 wt.% Mg, from 0.18 wt.% to 0.23 wt.% Fe, from 0.09 wt.% to 0.12 wt.% Si, from 0.05 wt.% to 0.15 wt.% Zr, from 0.04 wt.% to 0.09 wt.% Mn, from 0.03 wt.% to 0.09 wt.% Cr, from 0.01 wt.% to 0.02 wt.% Ti, up to 0.15 wt.% of impurities, and remainder Al. The rolled aluminum alloy product further includes up to 0.20 wt.% of one or more of Mo, Nb, Be, B, Co, Sn, Sr, V, In, Hf, Ag, Sc and Ni.

The methods described herein include heating the rolled aluminum alloy product to a first temperature of from 400 °C to 525 °C. For example, the first temperature may be from 450 °C to 510 °C. In some embodiments, the first temperature may be a solutionizing temperature. After heating the rolled aluminum alloy product to the first temperature, the rolled aluminum alloy product is maintained at the first temperature or within 10 °C of the first temperature for a time duration of from 15 seconds to 30 minutes. The method also includes quenching the rolled aluminum alloy product at a quench rate from 0.5 °C/s to 125 °C/s to generate a heat-treated aluminum alloy product. In some embodiments, the quench rate may be from 5 °C/s to 125 °C/s, while in other embodiments, the quench rate may be from 10 °C/s to 125 °C/s. Optionally, the quench rate may be from 5 °C/s to 10 °C/s, from 10 °C/s to 15 °C/s, from 15 °C/s to 20 °C/s, from 20 °C/s to 25 °C/s, from 25 °C/s to 30 °C/s, from 30 °C/s to 35 °C/s, from 35 °C/s to 40 °C/s, from 40 °C/s to 45 °C/s, from 45 °C/s to 50 °C/s, from 50 °C/s to 55 °C/s, from 55 °C/s to 60 °C/s, from 60 °C/s to 65 °C/s, from 65 °C/s to 70 °C/s, from 70 °C/s to 75 °C/s, from 75 °C/s to 80 °C/s, from 80 °C/s to 85 °C/s, from 85 °C/s to 90 °C/s, from 90 °C/s to 95 °C/s, from 95 °C/s to 100 °C/s, from 100 °C/s to 105 °C/s, from 105 °C/s to 110 °C/s, from 110 °C/s to 115 °C/s, from 115 °C/s to 120 °C/s, or from 120 °C/s to 125 °C/s.

In some embodiments, quenching the rolled aluminum alloy product may include a first quenching at a first quench rate to an intermediate temperature and a second quenching at a second quench rate to the second temperature. The second quench rate may be greater than the first quench rate. The rolled aluminum alloy product is quenched until the rolled aluminum alloy product reaches a second temperature of from 10 °C to 100°C. Optionally, the second temperature may be an ambient temperature. In some embodiments, quenching the rolled aluminum alloy product may include a die quenching process, a water quenching process, and/or a forced air quenching process. As an example, the first quench rate may correspond to or occur when the aluminum alloy product is removed from the heating system but before the product is introduced to the quenching system (e.g., a die quench). The initial drop in temperature due to exposure to ambient conditions may be or correspond to the first quench rate. Optionally, the second quenching may then correspond to the quenching that occurs during an active quenching process, such as a die quenching process.

Heating and quenching the rolled aluminum alloy product may correspond to a solutionizing heat treatment process, in some embodiments. Optionally, the method may further include subjecting the rolled aluminum alloy product to a hot forming process after heating the rolled aluminum alloy product. In some cases, the method may also include aging the heat-treated aluminum alloy product, such as in a T6 temper or T7 temper. For example, the heat-treated aluminum alloy product may optionally be further heated to a temperature from 100 °C to 170 °C and maintained at the temperature for 12 hours to 30 hours. Other aging and tempering processes, practices, and conditions may be utilized, such as those described in U.S. Patent Application publication US 2018/0202031.

The heat-treated aluminum alloy product may exhibit desirable and/or improved mechanical properties. For example, the heat-treated aluminum alloy product generated by quenching the rolled aluminum alloy product may exhibit a strain ratio of from 0.30 to 0.80. For example, the heat-treated aluminum alloy product may exhibit a strain ratio of from 0.375 to 0.425 when the quench rate is about or less than 125 °C/s. The strain ratio may be determined according to an ASTM G129 standard test method, such as ASTM G129-00(2013), Standard Practice for Slow Strain Rate Testing to Evaluate the Susceptibility of Metallic Materials to Environmentally Assisted Cracking, ASTM International, West Conshohocken, PA, 2013 or according to an ASTM G139 standard test method, such as ASTM G139-05(2015), Standard Test Method for Determining Stress-Corrosion Cracking Resistance of Heat-Treatable Aluminum Alloy Products Using Breaking Load Method, ASTM International, West Conshohocken, PA, 2015. In some embodiments, the heat-treated aluminum alloy product may exhibit an ultimate tensile strength of from 500 MPa to 650 MPa. For example, the heat-treated aluminum alloy product may exhibit an ultimate tensile strength of from 605 MPa to 615 MPa when the quench rate is about or less than 125 °C/s. In some embodiments, the heat-treated aluminum alloy product may exhibit a yield strength of from 400 MPa to 600 MPa. For example, the heat-treated aluminum alloy product may exhibit a yield strength of from 560 MPa to 580 MPa when the quench rate is about or less than 125 °C/s. In some embodiments, the heat-treated aluminum alloy product may exhibit a uniform elongation of from 7.50% to 10.50%. For example, the heat-treated aluminum alloy product may exhibit a uniform elongation of from 9.00% to 9.60% when the quench rate is about or less than 125 °C/s. In some embodiments, the heat-treated aluminum alloy product may exhibit a total elongation of from 10.00% to 15.00%. For example, the heat-treated aluminum alloy product may exhibit a total elongation of from 13.80% to 14.20% when the quench rate is about or less than 125 °C/s. In some embodiments, the heat-treated aluminum alloy product may exhibit precipitate-free zone widths from 10 nm to 110 nm. For example, the heat-treated aluminum alloy product may exhibit precipitate-free zone widths from 10 nm to 13 nm when the quench rate is about or less than 125 °C/s.

The heat-treated aluminum alloy product may also exhibit superior corrosion resistance. The heat-treated aluminum alloy product generated by quenching may exhibit a corrosion depth of from 5 µm to 300 µm as determined according to an ASTM G110 standard test method. For example, the heat-treated aluminum alloy product may exhibit a corrosion depth from 5 µm to 150 µm or from 25 µm to 50 µm when the quench rate is about 125 °C/s. In some cases, the corrosion depth may include at least one of pitting corrosion or intergranular corrosion. In some embodiments, the corrosion may include intergranular corrosion when the quench rate is about 50 °C/s or less. Optionally, the corrosion may not include intergranular corrosion when the quench rate is greater than or about 5 °C/s.

Optionally, the mechanical properties and corrosion resistance of the heat-treated aluminum alloy products may exceed those stated above when subjected to faster quenching, but it will be appreciated that quenching at rates of less than or about 125 °C/s may allow for more flexibility in handling and processing the hot aluminum alloy product immediately after heat-treatment without the final heat-treated aluminum alloy product suffering from poor mechanical properties or corrosion resistance. In this way, by using the aluminum alloy products described herein, the quenching process may be less complex and more forgiving and may simplify heat-treatment, quenching, stamping, or other processes.

A heat-treated aluminum alloy product is described herein, generated according to the method defined in the claims. The heat-treated aluminum alloy product includes a 7xxx series aluminum alloy product as defined in claim 1. In some embodiments, the heat-treated aluminum alloy product may be a formed aluminum alloy product, a hot formed aluminum alloy product, and/or in a T6 temper or T7 temper.

The product may be a heat-treated aluminum alloy product having improved mechanical properties. For example, the heat-treated aluminum alloy product may exhibit a strain ratio of from 0.30 to 0.80. For example, the heat-treated aluminum alloy product may exhibit a strain ratio of from 0.375 to 0.425 when a quench rate is less than or about 125 °C/s. The strain ratio may be determined according to an ASTM G129 and/or ASTM G139 standard test method. In some embodiments, the heat-treated aluminum alloy product may exhibit an ultimate tensile strength of from 500 MPa to 650 MPa, such as from 500 MPa to 510 MPa, 510 MPa to 520 MPa, 520 MPa to 530 MPa, 530 MPa to 540 MPa, 540 MPa to 550 MPa, 550 MPa to 560 MPa, 560 MPa to 570 MPa, 570 MPa to 580 MPa, 580 MPa to 590 MPa, 590 MPa to 600 MPa, 600 MPa to 610 MPa, 610 MPa to 620 MPa, 620 MPa to 630 MPa, 630 MPa to 640 MPa, or 640 MPa to 650 MPa. For example, the heat-treated aluminum alloy product may exhibit an ultimate tensile strength of from 605 MPa to 615 MPa when a quench rate is less than or about 125 °C/s. In some embodiments, the heat-treated aluminum alloy product may exhibit a yield strength of from 400 MPa to 600 MPa, such as from 400 MPa to 410 MPa, 410 MPa to 420 MPa, 420 MPa to 430 MPa, 430 MPa to 440 MPa, 440 MPa to 450 MPa, 450 MPa to 460 MPa, 460 MPa to 470 MPa, 470 MPa to 480 MPa, 480 MPa to 490 MPa, 490 MPa to 500 MPa, 500 MPa to 510 MPa, 510 MPa to 520 MPa, 520 MPa to 530 MPa, 530 MPa to 540 MPa, 540 MPa to 550 MPa, 550 MPa to 560 MPa, 560 MPa to 570 MPa, 570 MPa to 580 MPa, 580 MPa to 590 MPa, or 590 MPa to 600 MPa. For example, the heat-treated aluminum alloy product may exhibit a yield strength of from 560 MPa to 580 MPa when a quench rate is less than or about 125 °C/s. In some embodiments, the heat-treated aluminum alloy product may exhibit a uniform elongation of from 7.50% to 10.50%, such as from 7.50% to 8.00%, from 8.00% to 8.50%, from 8.50% to 9.00%, from 9.00% to 9.50%, from 9.50% to 10.00%, or from 10.00% to 10.50%. For example, the heat-treated aluminum alloy product may exhibit a uniform elongation of from 9.00% to 9.60% when a quench rate is less than or about 125 °C/s. In some embodiments, the heat-treated aluminum alloy product may exhibit a total elongation of from 10.00% to 15.00%, such as from 10.00% to 10.50%, from 10.50% to 11.00%, from 11.00% to 11.50%, from 11.50% to 12.00%, from 12.00% to 12.50%, from 12.50% to 13.00%, from 13.00% to 13.50%, from 13.50% to 14.00%, from 14.00% to 14.50%, or from 14.50% to 15.00%. For example, the heat-treated aluminum alloy product may exhibit a total elongation of from 13.80% to 14.20% when a quench rate is less than or about 125 °C/s. In some embodiments, the heat-treated aluminum alloy product may exhibit precipitate-free zone widths from 10 nm to 110 nm, such as from 10 nm to 11 nm, from 11 nm to 12 nm, from 12 nm to 13 nm, from 13 nm to 14 nm, from 14 nm to 15 nm, from 15 nm to 20 nm, from 20 nm to 25 nm, from 25 nm to 30 nm, from 30 nm to 35 nm, from 35 nm to 40 nm, from 40 nm to 45 nm, from 45 nm to 50 nm, from 50 nm to 55 nm, from 55 nm to 60 nm, from 60 nm to 65 nm, from 65 nm to 70 nm, from 70 nm to 75 nm, from 75 nm to 80 nm, from 80 nm to 85 nm, from 85 nm to 90 nm, from 90 nm to 95 nm, from 95 nm to 100 nm, from 100 nm to 105 nm, or from 105 nm to 110 nm. For example, the heat-treated aluminum alloy product may exhibit precipitate-free zone widths from 10 nm to 13 nm when a quench rate is less than or about 125 °C/s.

The product may include a heat-treated aluminum alloy product having superior corrosion resistance. For example, the heat-treated aluminum alloy product may exhibit a corrosion depth of from 5 µm to 300 µm as determined according to an ASTM G110 standard test method, such as from 5 µm to 10 µm, from 10 µm to 15 µm, from 15 µm to 20 µm, from 20 µm to 25 µm, from 25 µm to 30 µm, from 30 µm to 35 µm, from 35 µm to 40 µm, from 40 µm to 45 µm, from 45 µm to 50 µm, from 50 µm to 60 µm, from 60 µm to 70 µm, from 70 µm to 80 µm, from 80 µm to 90 µm, from 90 µm to 100 µm, from 100 µm to 110 µm, from 110 µm to 120 µm, from 120 µm to 130 µm, from 130 µm to 140 µm, from 140 µm to 150 µm, from 150 µm to 160 µm, from 160 µm to 170 µm, from 170 µm to 180 µm, from 180 µm to 190 µm, from 190 µm to 200 µm, from 200 µm to 210 µm, from 210 µm to 220 µm, from 220 µm to 230 µm, from 230 µm to 240 µm, from 240 µm to 250 µm, from 250 µm to 260 µm, from 260 µm to 270 µm, from 270 µm to 280 µm, from 280 µm to 290 µm, or from 290 µm to 300 µm. In some embodiments, the heat-treated aluminum alloy product may exhibit a corrosion depth from 5 µm to 150 µm or from 25 µm to 50 µm when a quench rate is less than or 125 °C/s.

The heat-treated aluminum alloy product is generated by heating a rolled aluminum alloy product to a first temperature. The rolled aluminum alloy product includes a 7xxx series aluminum alloy as defined in claim 1. The rolled aluminum alloy product is heated to a temperature from 400 °C to 525 °C. The rolled aluminum alloy product is maintained at the first temperature or within 10 °C of the first temperature for a time duration of from 15 seconds to 30 minutes, such as from 15 seconds to 30 seconds, from 30 seconds to 1 minute, from 1 minute to 5 minutes, from 5 minutes to 10 minutes, from 10 minutes to 15 minutes, from 15 minutes to 20 minutes, from 20 minutes to 25 minutes, or from 25 minutes to 30 minutes. The rolled aluminum alloy product is also quenched at a quench rate from 0.5 °C/s to 125 °C/s, such as from 0.5 °C/s to 1 °C/s, from 1 °C/s to 5 °C/s, from 5 °C/s to 10 °C/s, from 10 °C/s to 25 °C/s, from 25 °C/s to 50 °C/s, from 50 °C/s to 75 °C/s, from 75 °C/s to 100 °C/s, or from 100 °C/s to 125 °C/s. The product is generated by the methods described herein.

Automotive and aerospace products are also described herein. An automotive product may incorporate a product as described herein. For example, the automotive product may incorporate a heat-treated aluminum alloy product as described above. An aerospace product may incorporate a product as described herein. For example, the aerospace product may incorporate a heat-treated aluminum alloy product as described above. Optionally, an automotive product may incorporate a product generated according to any of the methods described herein. For example, the automotive product may incorporate a heat-treated aluminum alloy product generated by any of the methods described above. Similarly, an aerospace product may incorporate a product generated according to any of the methods described herein. For example, the aerospace product may incorporate a heat-treated aluminum alloy product generated by any of the methods described above.

Other objects and advantages will be apparent from the following detailed description of non-limiting examples.

### BRIEF DESCRIPTION OF THE FIGURES

The specification makes reference to the following appended figures, in which use of like reference numerals in different figures is intended to illustrate like or analogous components.
FIG. 1A provides a cross-sectional view of a corrosion profile of a quench-sensitive aluminum alloy product quenched at a rate of 550 °C/s.
FIG. 1B provides a cross-sectional view of a corrosion profile of a quench-sensitive aluminum alloy product quenched at a rate of 350 °C/s.
FIG. 1C provides a cross-sectional view of a corrosion profile of a quench-sensitive aluminum alloy product quenched at a rate of 250 °C/s.
FIG. 1D provides a cross-sectional view of a corrosion profile of a quench-sensitive aluminum alloy product quenched at a rate of 5 °C/s.
FIG. 2A provides a cross-sectional view of a corrosion profile of a heat-treated aluminum alloy product quenched at a rate of 550 °C/s according to an embodiment.
FIG. 2B provides a cross-sectional view of a corrosion profile of a heat-treated aluminum alloy product quenched at a rate of 350 °C/s according to an embodiment.
FIG. 2C provides a cross-sectional view of a corrosion profile of a heat-treated aluminum alloy product quenched at a rate of 250 °C/s according to an embodiment.
FIG. 2D provides a cross-sectional view of a corrosion profile of a heat-treated aluminum alloy product quenched at a rate of 5 °C/s according to an embodiment.
FIG. 3A provides a cross-sectional view of a corrosion profile of a heat-treated aluminum alloy product quenched at a rate of 550 °C/s according to another embodiment.
FIG. 3B provides a cross-sectional view of a corrosion profile of a heat-treated aluminum alloy product quenched at a rate of 350 °C/s according to another embodiment.
FIG. 3C provides a cross-sectional view of a corrosion profile of a heat-treated aluminum alloy product quenched at a rate of 250 °C/s according to another embodiment.
FIG. 3D provides a cross-sectional view of a corrosion profile of a heat-treated aluminum alloy product quenched at a rate of 5 °C/s according to another embodiment.
FIG. 4 provides an illustrative graph showing a comparison of corrosion depths at different quench rates for a quench-sensitive aluminum alloy product versus heat-treated aluminum alloy products made according to some embodiments.
FIG. 5 provides an illustrative graph showing a comparison of yield strengths at different quench rates for a quench-sensitive aluminum alloy product versus heat-treated aluminum alloy products made according to some embodiments.
FIG. 6 provides an illustrative graph showing a comparison of ultimate tensile strengths at different quench rates for a quench-sensitive aluminum alloy product versus heat-treated aluminum alloy products made according to some embodiments.
FIG. 7 provides an illustrative graph showing a comparison of total elongation at different quench rates for a quench-sensitive aluminum alloy product versus heat-treated aluminum alloy products made according to some embodiments.
FIG. 8 provides an illustrative graph showing a comparison of strain ratios at different quench rates for a quench-sensitive aluminum alloy product versus a heat-treated aluminum alloy product made according to some embodiments.
FIG. 9 provides an illustrative graph showing a comparison of precipitate-free zone widths at different quench rates for a quench-sensitive aluminum alloy product versus heat-treated aluminum alloy products made according to some embodiments.
FIG. 10A provides an electron micrograph image showing precipitate-free zones formed when a quench-sensitive aluminum alloy product is quenched at a rate of 550 °C/s.
FIG. 10B provides an electron micrograph image showing precipitate-free zones formed when a quench-sensitive aluminum alloy product is quenched at a rate of 150 °C/s.
FIG. 10C provides an electron micrograph image showing precipitate-free zones formed when a quench-sensitive aluminum alloy product is quenched at a rate of 5 °C/s.
FIG. 11A provides an electron micrograph image showing precipitate-free zones of a heat-treated aluminum alloy product formed when a rolled aluminum alloy product made according to embodiments disclosed herein is quenched at a rate of 550 °C/s.
FIG. 11B provides an electron micrograph image showing precipitate-free zones of a heat-treated aluminum alloy product formed when a rolled aluminum alloy product made according to embodiments disclosed herein is quenched at a rate of 150 °C/s.
FIG. 11C provides an electron micrograph image showing precipitate-free zones of a heat-treated aluminum alloy product formed when a rolled aluminum alloy product made according to embodiments disclosed herein is quenched at a rate of 5 °C/s.
FIG. 12 provides an overview of a method of making an aluminum alloy product according to some embodiments.
FIG. 13 provides an illustrative graph showing the temperature profile as a function of time for making aluminum alloy products according to some embodiments.

### DETAILED DESCRIPTION

Described herein are aluminum alloy products and methods of making aluminum alloy products processed in a way that achieves improved quench sensitivity. Quench sensitivity commonly refers to the impact of quenching on a metal product's properties, such as mechanical properties and corrosion resistance. Quenching refers to a rapid cooling of a metal product from a first temperature, such as a heat treatment temperature, to a lower temperature, such as room temperature. During processing, aluminum alloy products undergo a heat treatment in which the aluminum alloy product is heated to a first high temperature, such as from 450 °C to 525 °C. The aluminum alloy products may be subjected to heat treatments, such as those described in U.S. patent application Ser. No. 15/336,982. One objective of quenching is to preserve a metastable solid solution formed by the heat treatment. When a product is cooled at a sufficient rate from the first temperature to a second temperature, often near or at room temperature, a solid solution in which solutes remain in the alloy solution may be achieved. Solute retention may be desirable because precipitation of the solute out of solution during quenching can lead to localized overaging, loss of grain-boundary corrosion resistance, and, importantly, poor response to age hardening treatments. Retention of the solute in the solid solution may allow for solute atoms to be available to form zones of homogenous precipitation which are important for strengthening the metal product during age hardening treatments. Another goal of quenching may be to maintain a desirable number of vacant lattice sites to assist in promoting low-temperature diffusion during the aging stage of precipitation hardening.

Some metal products, such as aluminum alloy products, may be particularly sensitive to solute loss. Particularly during age hardening treatments, solute loss may affect the resulting properties of an aluminum alloy product. Solute loss refers to the solutes that are chemically bonded with other elements, rendering them unavailable for precipitation hardening. When quench rates are not sufficiently rapid, then solute atoms are prone to diffuse to the grain boundaries, as well as the vacancies that migrate to disordered regions. Such movement of solute atoms is often irretrievable and may permanently affect the properties of the metal product. For example, some metal products that are not quenched at a sufficient rate may exhibit higher rates of intergranular corrosion and stress cracking corrosion, and have reduced yield strength, tensile strength, and grain elongation. Accordingly, the most desirable mechanical properties attainable may be generally associated with high quench rates.

However, achieving high quench rates may be costly, complex, or require time-sensitive processes which minimize opportunity for additional processing between heat treatment steps and quenching steps. Moreover, high quench rates may undesirably affect a metal product's properties. High quench rates may also result in distortion and development of residual stress within the microstructure of the product, in some cases. Aluminum alloy products may be prone to distortion during quenching due to aluminum's high linear expansion coefficient, for example. The coefficient of linear expansion of aluminum is twice that of steel and thus, during large temperature swings, significant amounts of strain can develop due to thermal expansion or contraction. Accordingly, a balance between a quench rate that sufficiently retains most of the hardening elements and compounds in solution and minimizes distortion and residual stress may be desirable to make an aluminum alloy product having optimal properties.

One approach to balancing the effects of quenching involves multi-step aging processes. Often these multi-step aging processes include at least one rapid quench step. For example, the initial quench from the first temperature may be rapid to maintain the solid solution. However, multi-step aging processes may be complex, costly, and time consuming. Accordingly, as described herein, methods and metal products are provided for achieving desirable properties using only a single step aging process, despite use of smaller quench rates. Additionally, the disclosed methods and metal products may exhibit quench insensitivity, resulting in improved mechanical properties, such as improved strength values, even at low quench rates.

In particular, the disclosed methods and techniques may provide for quench-insensitive 7xxx series aluminum alloys and products subjected to only a single step aging process. The quench-insensitive 7xxx series aluminum alloys described herein may have improved intergranular corrosion and stress corrosion cracking resistance without rapid quenching. Exemplary 7xxx series aluminum alloys for use in the disclosed methods and techniques are described in U.S. Patent Application No. 15/336,982.

### Definitions and Descriptions

As used herein, the terms "invention," "the invention," "this invention" and "the present invention" are intended to refer to the invention as disclosed in the claims below.

In this description, reference is made to alloys identified by AA numbers and other related designations, such as "series" or "7xxx." For an understanding of the number designation system most commonly used in naming and identifying aluminum and its alloys, see "International Alloy Designations and Chemical Composition Limits for Wrought Aluminum and Wrought Aluminum Alloys" or "Registration Record of Aluminum Association Alloy Designations and Chemical Compositions Limits for Aluminum Alloys in the Form of Castings and Ingot," both published by The Aluminum Association.

As used herein, a plate generally has a thickness of greater than about 15 mm. For example, a plate may refer to an aluminum product having a thickness of greater than about 15 mm, greater than about 20 mm, greater than about 25 mm, greater than about 30 mm, greater than about 35 mm, greater than about 40 mm, greater than about 45 mm, greater than about 50 mm, or greater than about 100 mm.

As used herein, a shate (also referred to as a sheet plate) generally has a thickness of from about 4 mm to about 15 mm. For example, a shate may have a thickness of about 4 mm, about 5 mm, about 6 mm, about 7 mm, about 8 mm, about 9 mm, about 10 mm, about 11 mm, about 12 mm, about 13 mm, about 14 mm, or about 15 mm.

As used herein, a sheet generally refers to an aluminum product having a thickness of less than about 4 mm. For example, a sheet may have a thickness of less than about 4 mm, less than about 3 mm, less than about 2 mm, less than about 1 mm, less than about 0.5 mm, or less than about 0.3 mm (e.g., about 0.2 mm).

Reference may be made in this application to alloy temper or condition. For an understanding of the alloy temper descriptions most commonly used, see "American National Standards (ANSI) H35 on Alloy and Temper Designation Systems." An F condition or temper refers to an aluminum alloy as fabricated. An O condition or temper refers to an aluminum alloy after annealing. An Hxx condition or temper, also referred to herein as an H temper, refers to a non-heat treatable aluminum alloy after cold rolling with or without thermal treatment (e.g., annealing). Suitable H tempers include HX1, HX2, HX3 HX4, HX5, HX6, HX7, HX8, or HX9 tempers. A T1 condition or temper refers to an aluminum alloy cooled from hot working and naturally aged (e.g., at room temperature). A T2 condition or temper refers to an aluminum alloy cooled from hot working, cold worked and naturally aged. A T3 condition or temper refers to an aluminum alloy solution heat treated, cold worked, and naturally aged. A T4 condition or temper refers to an aluminum alloy solution heat treated and naturally aged. A T5 condition or temper refers to an aluminum alloy cooled from hot working and artificially aged (at elevated temperatures). A T6 condition or temper refers to an aluminum alloy solution heat treated and artificially aged. A T7 condition or temper refers to an aluminum alloy solution heat treated and artificially overaged. A T8x condition or temper refers to an aluminum alloy solution heat treated, cold worked, and artificially aged. A T9 condition or temper refers to an aluminum alloy solution heat treated, artificially aged, and cold worked. A W condition or temper refers to an aluminum alloy after solution heat treatment.

As used herein, the meaning of "room temperature" can include a temperature of from about 15 °C to about 30 °C, for example about 15 °C, about 16 °C, about 17 °C, about 18 °C, about 19 °C, about 20 °C, about 21 °C, about 22 °C, about 23 °C, about 24 °C, about 25 °C, about 26 °C, about 27 °C, about 28 °C, about 29 °C, or about 30 °C. As used herein, the meaning of "ambient conditions" or "ambient environment" can include temperatures of about room temperature, relative humidity of from about 20% to about 100%, and barometric pressure of from about 975 millibar (mbar) to about 1050 mbar. For example, relative humidity can be about 20%, about 21%, about 22%, about 23%, about 24%, about 25%, about 26%, about 27%, about 28%, about 29%, about 30%, about 31%, about 32%, about 33%, about 34%, about 35%, about 36%, about 37%, about 38%, about 39%, about 40%, about 41%, about 42%, about 43%, about 44%, about 45%, about 46%, about 47%, about 48%, about 49%, about 50%, about 51%, about 52%, about 53%, about 54%, about 55%, about 56%, about 57%, about 58%, about 59%, about 60%, about 61%, about 62%, about 63%, about 64%, about 65%, about 66%, about 67%, about 68%, about 69%, about 70%, about 71%, about 72%, about 73%, about 74%, about 75%, about 76%, about 77%, about 78%, about 79%, about 80%, about 81%, about 82%, about 83%, about 84%, about 85%, about 86%, about 87%, about 88%, about 89%, about 90%, about 91%, about 92%, about 93%, about 94%, about 95%, about 96%, about 97%, about 98%, about 99%, about 100%, or anywhere in between. For example, barometric pressure can be about 975 mbar, about 980 mbar, about 985 mbar, about 990 mbar, about 995 mbar, about 1000 mbar, about 1005 mbar, about 1010 mbar, about 1015 mbar, about 1020 mbar, about 1025 mbar, about 1030 mbar, about 1035 mbar, about 1040 mbar, about 1045 mbar, about 1050 mbar, or anywhere in between.

All ranges disclosed herein are to be understood to encompass any and all subranges subsumed therein. For example, a stated range of "1 to 10" should be considered to include any and all subranges between (and inclusive of) the minimum value of 1 and the maximum value of 10; that is, all subranges beginning with a minimum value of 1 or more, e.g., 1 to 6.1, and ending with a maximum value of 10 or less, e.g., 5.5 to 10. Unless stated otherwise, the expression "up to" when referring to the compositional amount of an element means that element is optional and includes a zero percent composition of that particular element. Unless stated otherwise, all compositional percentages are in weight percent (wt.%).

As used herein, the meaning of "a," "an," and "the" includes singular and plural references unless the context clearly dictates otherwise.

In the present description, aluminum alloy products and their components are described in terms of their elemental composition in weight percent (wt.%). In each alloy, the remainder is aluminum, with a maximum wt.% of 0.15% for the sum of all impurities.

### Aluminum Alloy Products and Methods of Making Aluminum Alloy Products

FIGs. 1A, 1B, 1C, and 1D provide cross-sectional views of a corrosion profile for a quench-sensitive aluminum alloy product quenched at various quench rates. A quench-sensitive aluminum alloy product may be a product made according to conventional methods and techniques. Corrosion profiles may be generated by subjecting the aluminum alloy product to a heat treatment process, followed by quenching at the indicated rate, and then subjecting the quenched aluminum alloy product to a standard corrosion test for determining or evaluating corrosion resistance, such as the American Society for Testing and Materials (ASTM) G139 Standard Test Method for Determining Stress-Corrosion Cracking Resistance or ASTM G110 Standard Practice for Evaluating Intergranular Corrosion Resistance of Heat Treatable Aluminum Alloys by Immersion in Sodium Chloride + Hydrogen Peroxide Solution. The corrosion profile may be obtained by sectioning the tested product and obtaining a cross sectional micrograph image.

For example, FIGs. 1A-1D depict a corrosion profile for a quench-sensitive aluminum alloy product identified as aluminum alloy product 110. Aluminum alloy product 110 may be an AA7075 aluminum alloy product. Other exemplary quench-sensitive aluminum alloy products 110 may include AA7022, AA7185, AA6056, AA7020, AA7049, AA7249, or AA7149. Although the discussion herein for FIGs. 1A-1D, FIGs. 2A-2D, and FIGs. 3A-3D describes aluminum alloy products, the figures and related discussion may also be applicable to other types of metal products, in general.

In embodiments, quench sensitivity may be determined based on quench rate and the type of corrosion exhibited by the aluminum alloy product upon corrosion testing. During corrosion testing of quenched products, various types of corrosion may be exhibited. For example, pitting corrosion may be exhibited in which cavities or holes, representing material loss, are formed within the aluminum alloy. In other examples, intergranular corrosion may be exhibited. Intergranular corrosion, also known as intercrystalline corrosion or interdendritic corrosion, may be characterized as a form of localized corrosion in which grain boundaries and material immediately adjacent to the grain boundaries are attacked. In some cases, quench sensitivity may be determined based on the form of corrosion and/or the transition from one form of corrosion to another. For example, quench sensitivity may correspond to a change in corrosion morphology, such as a switch from pitting corrosion to intergranular corrosion when a product is subjected to various quench rates. In some cases, the slower an aluminum alloy product may be quenched without exhibiting intergranular corrosion in a corrosion test, the more quench-insensitive the aluminum alloy product may be. Intergranular corrosion may be more undesirable than pitting corrosion because of the ability of intergranular corrosion to more easily propagate cracks under stress conditions.

As illustrated in FIG. 1A, when a quench-sensitive aluminum alloy product is quenched at a rapid quench rate of 550 °C/s pitting corrosion 120 may be exhibited in a corrosion test. Pitting corrosion 120 may be identified by localized pockets of material loss from the aluminum alloy product 110. Aluminum alloy product 110 may be quenched using water quenching to achieve the rapid quench rate of 550 °C/s. Water is commonly used for quenching aluminum alloy products. Common methods of water quenching may include cold water immersion, hot water immersion, boiling water, or water spray. Other quench methods also frequently used include polyalkylene glycol solutions, air blasts, still air (i.e., holding the aluminum alloy product at room temperature), liquid nitrogen, fast quenching oils, or brine solutions. Depending on the aluminum alloy product, desired properties, and required quenching rates, various quench methods may be selected.

FIG. 1B illustrates that pitting corrosion 120 may also be exhibited when aluminum alloy product 110 is quenched at a rate of 350 °C/s and subjected to a corrosion test. The corrosion morphology changes between FIG. 1B and FIG. 1C. As shown in the corrosion profile of FIG. 1C, intergranular corrosion 130 may be exhibited when aluminum alloy product 110 is quenched at a rate of 250 °C/s or below and subjected to a corrosion test. Intergranular corrosion 130 may be identified by formation of localized fracturing along the grain boundaries of aluminum alloy product 110. In corrosion profiles, such as those provided in FIGs. 1A-1D, intergranular corrosion 130 may be identified by slightly more delicate fracturing within the bulk of aluminum alloy product 110 as compared to large fracturing or pockets of material loss exhibited by pitting corrosion 120. Intergranular corrosion 130 may also be exhibited when aluminum alloy product 110 is quenched at a rate of 5 °C/s and subjected to a corrosion test. The change in corrosion morphology from pitting corrosion 120 to intergranular corrosion 130 between the quench rates of 350 °C/s and 250 °C/s may indicate that aluminum alloy product 110 is quench sensitive or requires a high quench rate to achieve resistance to intergranular corrosion. Moreover, this quench sensitivity of aluminum alloy product 110 may indicate that aluminum alloy product 110 may have fewer desirable properties, such as reduced stress corrosion cracking resistance or reduced strength values.

FIGs. 2A-2D provide corrosion profiles for a heat-treated aluminum alloy product according to methods and techniques disclosed herein. The heat-treated aluminum alloy products provided herein may be quench-insensitive aluminum alloy products. In FIGs. 2A-2D, the heat-treated aluminum alloy product is identified as aluminum alloy product 210. Aluminum alloy product 210 may be or comprise a 7xxx series aluminum alloy as described herein. These alloys may exhibit improved quench insensitivity and unexpectedly high strength values after quenching, such as high tensile and yield strengths, which may be maintained when subjected to corrosion testing. The properties of the aluminum alloy products disclosed herein may be achieved due to their compositions and the methods by which they are made and processed. Advantageously, the final properties of these aluminum alloy products may be achieved while undergoing a single step aging treatment. Additionally, the aluminum alloy products may be relatively quench insensitive, meaning that they can be quenched at slower quench rates without resulting in undesirable changes to properties, allowing for additional processing time between the heat treatment process and the quenching process, reduced quenching costs, and/or reduced distortion. An aluminum alloy as described herein may optionally have an elemental composition as provided in Table 1 (not according to the invention).

**Table 1.**

| Element | Weight Percentage (wt.%) |
|---|---|
| Zn | 4.00 - 15.00 |
| Cu | 0.10 - 3.50 |
| Mg | 1.00 - 4.00 |
| Fe | 0.05 - 0.50 |
| Si | 0.05 - 0.30 |
| Zr | 0.05 - 0.25 |
| Mn | 0.00 - 0.25 |
| Cr | 0.00 - 0.20 |
| Ti | 0.00 - 0.15 |
| Others | 0.00 - 0.05 (each) |
| | 0.00 - 0.15 (total) |
| Al | Remainder |

An aluminum alloy as described herein may have an elemental composition as provided in Table 2 (not according to the invention).

**Table 2.**

| Element | Weight Percentage (wt.%) |
|---|---|
| Zn | 5.60 - 9.30 |
| Cu | 0.20 - 2.60 |
| Mg | 1.40 - 2.80 |
| Fe | 0.10 - 0.35 |
| Si | 0.05 - 0.20 |
| Zr | 0.05 - 0.15 |
| Mn | 0.01 - 0.05 |
| Cr | 0.01 - 0.05 |
| Ti | 0.001 - 0.05 |
| Others | 0.00 - 0.05 (each) |
| | 0.00 - 0.15 (total) |
| Al | Remainder |

An aluminum alloy as described herein may have an elemental composition as provided in Table 3 (not according to the invention).

**Table 3.**

| Element | Weight Percentage (wt.%) |
|---|---|
| Zn | 5.80 - 9.20 |
| Cu | 0.30 - 2.50 |
| Mg | 1.60 - 2.60 |
| Fe | 0.10 - 0.25 |
| Si | 0.07 - 0.15 |
| Zr | 0.09 - 0.15 |
| Mn | 0.02 - 0.05 |
| Cr | 0.03 - 0.05 |
| Ti | 0.003 - 0.035 |
| Others | 0.00 - 0.05 (each) |
| | 0.00 - 0.15 (total) |
| Al | Remainder |

An aluminum alloy as described herein may have an elemental composition as provided in Table 4 (not according to the invention).

**Table 4**

| Element | Weight Percentage (wt.%) |
|---|---|
| Zn | 8.90 - 9.20 |
| Cu | 0.20 - 2.10 |
| Mg | 2.20 - 2.40 |
| Fe | 0.18 - 0.23 |
| Si | 0.09 - 0.12 |
| Zr | 0.05 - 0.15 |
| Mn | 0.04 - 0.09 |
| Cr | 0.03 - 0.09 |
| Ti | 0.01 - 0.02 |
| Others | 0.00 - 0.05 (each) |
| | 0.00 - 0.15 (total) |
| Al | Remainder |

The alloys described herein include zinc (Zn) in an amount of from 4.00% to 15.00% (e.g., from 5.40% to 9.50%, from 5.60% to 9.30%, from 5.80% to 9.20%, or from 4.00% to 5.00%) based on the total weight of the alloy. For example, the alloy may include 4.00%, 4.10%, 4.20%, 4.30%, 4.40%, 4.50%, 4.60%, 4.70%, 4.80%, 4.90%, 5.00%, 5.10%, 5.20%, 5.30%, 5.40%, 5.50%, 5.60%, 5.70%, 5.80%, 5.90%, 6.00%, 6.10%, 6.20%, 6.30%, 6.40%, 6.50%, 6.60%, 6.70%, 6.80%, 6.90%, 7.00%, 7.10%, 7.20%, 7.30%, 7.40%, 7.50%, 7.60%, 7.70%, 7.80%, 7.90%, 8.00%, 8.10%, 8.20%, 8.30%, 8.40%, 8.50%, 8.60%, 8.70%, 8.80%, 8.90%, 9.00%, 9.10%, 9.20%, 9.30%, 9.40%, 9.50%, 9.60%, 9.70%, 9.80%, 9.90%, 10.00%, 10.10%, 10.20%, 10.30%, 10.40%, 10.50%, 10.60%, 10.70%, 10.80%, 10.90%, 11.00%, 11.10%, 11.20%, 11.30%, 11.40%, 11.50%, 11.60%, 11.70%, 11.80%, 11.90%, 12.00%, 12.10%, 12.20%, 12.30%, 12.40%, 12.50%, 12.60%, 12.70%, 12.80%, 12.90%, 13.00%, 13.10%, 13.20%, 13.30%, 13.40%, 13.50%, 13.60%, 13.70%, 13.80%, 13.90%, 14.00%, 14.10%, 14.20%, 14.30%, 14.40%, 14.50%, 14.60%, 14.70%, 14.80%, 14.90%, or 15.00% Zn. Optionally, the alloy may include from 4.00% to 4.10%, from 4.10% to 4.20%, from 4.20% to 4.30%, from 4.30% to 4.40%, from 4.40% to 4.50%, from 4.50% to 4.60%, from 4.60% to 4.70%, from 4.70% to 4.80%, from 4.80% to 4.90%, from 4.90% to 5.00%, from 5.00% to 5.10%, from 5.10% to 5.20%, from 5.20% to 5.30%, from 5.30% to 5.40%, from 5.40% to 5.50%, from 5.50% to 5.60%, from 5.60% to 5.70%, from 5.70% to 5.80%, from 5.80% to 5.90%, from 5.90% to 6.00%, from 6.00% to 6.10%, from 6.10% to 6.20%, from 6.20% to 6.30%, from 6.30% to 6.40%, from 6.40% to 6.50%, from 6.50% to 6.60%, from 6.60% to 6.70%, from 6.70% to 6.80%, from 6.80% to 6.90%, from 6.90% to 7.00%, from 7.00% to 7.10%, from 7.10% to 7.20%, from 7.20% to 7.30%, from 7.30% to 7.40%, from 7.40% to 7.50%, from 7.50% to 7.60%, from 7.60% to 7.70%, from 7.70% to 7.80%, from 7.80% to 7.90%, from 7.90% to 8.00%, from 8.00% to 8.10%, from 8.10% to 8.20%, from 8.20% to 8.30%, from 8.30% to 8.40%, from 8.40% to 8.50%, from 8.50% to 8.60%, from 8.60% to 8.70%, from 8.70% to 8.80%, from 8.80% to 8.90%, from 8.90% to 9.00%, from 9.00% to 9.10%, from 9.10% to 9.20%, from 9.20% to 9.30%, from 9.30% to 9.40%, from 9.40% to 9.50%, from 9.50% to 9.60%, from 9.60% to 9.70%, from 9.70% to 9.80%, from 9.80% to 9.90%, from 9.90% to 10.00%, from 10.00% to 10.10%, from 10.10% to 10.20%, from 10.20% to 10.30%, from 10.30% to 10.40%, from 10.40% to 10.50%, from 10.50% to 10.60%, from 10.60% to 10.70%, from 10.70% to 10.80%, from 10.80% to 10.90%, from 10.90% to 11.00%, from 11.00% to 11.10%, from 11.10% to 11.20%, from 11.20% to 11.30%, from 11.30% to 11.40%, from 11.40% to 11.50%, from 11.50% to 11.60%, from 11.60% to 11.70%, from 11.70% to 11.80%, from 11.80% to 11.90%, from 11.90% to 12.00%, from 12.00% to 12.10%, from 12.10% to 12.20%, from 12.20% to 12.30%, from 12.30% to 12.40%, from 12.40% to 12.50%, from 12.50% to 12.60%, from 12.60% to 12.70%, from 12.70% to 12.80%, from 12.80% to 12.90%, from 12.90% to 13.00%, from 13.00% to 13.10%, from 13.10% to 13.20%, from 13.20% to 13.30%, from 13.30% to 13.40%, from 13.40% to 13.50%, from 13.50% to 13.60%, from 13.60% to 13.70%, from 13.70% to 13.80%, from 13.80% to 13.90%, from 13.90% to 14.00%, from 14.00% to 14.10%, from 14.10% to 14.20%, from 14.20% to 14.30%, from 14.30% to 14.40%, from 14.40% to 14.50%, from 14.50% to 14.60%, from 14.60% to 14.70%, from 14.70% to 14.80%, from 14.80% to 14.90%, or from 14.90% to 15.00% Zn. All are expressed in wt.%.

The alloys described include copper (Cu) in an amount of from 0.30% to 2.50% or from 0.20% to 2.10% based on the total weight of the alloy. For example, the alloy may include 0.20%, 0.21%, 0.22%, 0.23%, 0.24%, 0.25%, 0.26%, 0.27%, 0.28%, 0.29%, 0.30%, 0.35%, 0.4%, 0.45%, 0.50%, 0.55%, 0.60%, 0.65%, 0.70%, 0.75%, 0.80%, 0.85%, 0.90%, 0.95%, 1.0%, 1.1%, 1.2%, 1.3%, 1.4%, 1.5%, 1.6%, 1.7%, 1.8%, 1.9%, 2.0%, 2.1%, 2.2%, 2.3%, 2.4%, or 2.5% Cu. Optionally, the alloy may include from 0.20% to 0.21%, from 0.21% to 0.22%, from 0.22% to 0.23%, from 0.23% to 0.24%, from 0.24% to 0.25%, from 0.25% to 0.26%, from 0.26% to 0.27%, from 0.27% to 0.28%, from 0.28% to 0.29%, from 0.29% to 0.30%, from 0.30% to 0.35%, from 0.35% to 0.40%, from 0.40% to 0.45%, from 0.45% to 0.50%, from 0.50% to 0.55%, from 0.55% to 0.60%, from 0.60% to 0.65%, from 0.65% to 0.70%, from 0.70% to 0.75%, from 0.75% to 0.80%, from 0.80% to 0.85%, from 0.85% to 0.90%, from 0.90% to 0.95%, from 0.95% to 1.0%, from 1.0% to 1.1%, from 1.1% to 1.2%, from 1.2% to 1.3%, from 1.3% to 1.4%, or from 1.4% to 1.5% Cu.
All are expressed in wt.%.

The alloys described herein include magnesium (Mg) in an amount of from 1.60% to 2.60% or from 2.20% to 2.40%. In some cases, the alloy can include 1.60%, 1.70%, 1.80%, 1.90%, 2.00%, 2.10%, 2.20%, 2.30%, 2.40%, 2.50%, or 2.60% Mg. Optionally, the alloy can include from 1.60% to 1.70%, from 1.80% to 1.80%, from 1.80% to 1.90%, from 1.90% to 2.00%, from 2.00% to 2.10%, from 2.10% to 2.20%, from 2.20% to 2.30%, from 2.30% to 2.40%, from 2.40% to 2.50%, or from 2.50% to 2.60% Mg. All are expressed in wt.%.

Optionally, the combined content of Zn, Cu, and Mg may range from 5.00% to 14.00% (e.g., from 5.50% to 13.50%, from 6.00% to 13.00%, from 6.50% to 12.50%, or from 7.00% to 12.00%). For example, the combined content of Zn, Cu, and Mg may be 5.00%, 5.50%, 6.00%, 6.50%, 7.00%, 7.50%, 8.00%, 8.50%, 9.00%, 9.50%, 10.00%, 10.50%, 11.00%, 11.50%, 12.00%, 12.50%, 13.00%, 13.50%, or 14.00%. Optionally, the combined content of Zn, Cu, and Mg may be from 5.00% to 5.50%, from 5.50% to 6.00%, from 6.00% to 6.50%, from 6.50% to 7.00%, from 7.00% to 7.50%, from 7.50% to 8.00%, from 8.00% to 8.50%, from 8.50% to 9.00%, from 9.00% to 9.50%, from 9.50% to 10.00%, from 10.00% to 10.50%, from 10.50% to 11.00%, from 11.00% to 11.50%, from 11.50% to 12.00%, from 12.00% to 12.50%, from 12.50% to 13.00%, from 13.00% to 13.50%, or from 13.50% to 14.00%. All are expressed in wt.%.

The alloys described herein include iron (Fe) in an amount of from 0.10% to 0.25% or from 0.18% to 0.23% based on the total weight of the alloy. For example, the alloy may include 0.10%, 0.11%, 0.12%, 0.13%, 0.14%, 0.15%, 0.16%, 0.17%, 0.18%, 0.19%, 0.20%, 0.21%, 0.22%, 0.23%, 0.24%, or 0.25%Fe. Optionally, the alloy may include from 0.10% to 0.11%, from 0.11% to 0.12%, from 0.12% to 0.13%, from 0.13% to 0.14%, from 0.14% to 0.15%, from 0.15% to 0.16%, from 0.16% to 0.17%, from 0.17% to 0.18%, from 0.18% to 0.19%, from 0.19% to 0.20%, from 0.20% to 0.21%, from 0.21% to 0.22%, from 0.22% to 0.23%, from 0.23% to 0.24%, or from 0.24% to 0.25%
Fe. All are expressed in wt.%.

The alloys described herein include silicon (Si) in an amount of from 0.07% to 0.15% or from 0.09% to 0.12% based on the total weight of the alloy. For example, the alloy may include 0.07%, 0.08%, 0.09%, 0.10%, 0.11%, 0.12%, 0.13%, 0.14%, or 0.15% Si. Optionally, the alloy may include from 0.07% to 0.08%, from 0.08% to 0.09%, from 0.09% to 0.10%, from 0.10% to 0.11%, from 0.11% to 0.12%, from 0.12% to 0.13%, from 0.13% to 0.14%, or from 0.14% to 0.15% Si. All are expressed in wt.%.

The alloys described herein include zirconium (Zr) in an amount of from 0.09% to 0.15% or from 0.05% to 0.15% based on the total weight of the alloy. For example, the alloy may include 0.05%, 0.06%, 0.07%, 0.08%, 0.09%, 0.10%, 0.11%, 0.12%, 0.13%, 0.14%, or 0.15% Zr. Optionally, the alloy may include from 0.05% to 0.06%, from 0.06% to 0.07%, from 0.07% to 0.08%, from 0.08% to 0.09%, from 0.09% to 0.10%, from 0.10% to 0.11%, from 0.11% to 0.12%, from 0.12% to 0.13%, from 0.13% to 0.14%, or from 0.14% to 0.15% Zr. All are expressed in wt.%.

The alloys described herein include manganese (Mn) in an amount from 0.02% to 0.05% or 0.04% to 0.09% based on the total weight of the alloy. For example, the alloy may include 0.02%, 0.03%, 0.04%, 0.05%, 0.06%, 0.07%, 0.08%, or 0.09% Mn. Optionally, the alloy may include from 0.02% to 0.03%, from 0.03% to 0.04%, from 0.04% to 0.05%, from 0.05% to 0.06%, from 0.06% to 0.07%, from 0.07% to 0.08%, or from 0.08% to 0.09% Mn. All are expressed in wt.%.

The alloys described herein include chromium (Cr) in an amount from 0.03% to 0.05% or from 0.03% to 0.09% based on the total weight of the alloy. For example, the alloy may include 0.03%, 0.04%, 0.05%, 0.06%, 0.07%, 0.08%, or 0.09% Cr. Optionally, the alloy may include from 0.03% to 0.04%, from 0.04% to 0.05%, from 0.05% to 0.06%, from 0.06% to 0.07%, from 0.07% to 0.08%, or from 0.08% to 0.09% Cr. All are expressed in wt.%.

The alloys described herein include titanium (Ti) in an amount from 0.003% to 0.035% or from 0.01% to 0.02% based on the total weight of the alloy. For example, the alloy may include 0.003%, 0.004%, 0.005%, 0.006%, 0.007%, 0.008%, 0.009%, 0.010%, 0.011% 0.012%, 0.013%, 0.014%, 0.015%, 0.016%, 0.017%, 0.018%, 0.019%, 0.020%, 0.021% 0.022%, 0.023%, 0.024%, 0.025%, 0.026%, 0.027%, 0.028%, 0.029%,0.03%, 0.031% 0.032%, 0.033%, 0.034%, or 0.035% Ti. Optionally, the alloy may include from 0.01% to 0.02%, or from 0.02% to 0.03% Ti. All are expressed in wt.%.

The alloys described herein may include one or more of Mo, Nb, Be, B, Co, Sn, Sr, V, In, Hf, Ag, and Ni in an amount of up to 0.20% (e.g., from 0.01% to 0.20% or from 0.05% to 0.15%) based on the total weight of the alloy. For example, the alloy may include 0.05%, 0.06%, 0.07%, 0.08%, 0.09%, 0.10%, 0.11%, 0.12%, 0.13%, 0.14%, 0.15%, 0.16%, 0.17%, 0.18%, 0.19%, or 0.20% of one or more of Mo, Nb, Be, B, Co, Sn, Sr, V, In, Hf, Ag, and Ni. Optionally, the alloy may include from 0.01% to 0.02%, from 0.02% to 0.03%, from 0.03% to 0.04%, from 0.04% to 0.05%, from 0.05% to 0.06%, from 0.06% to 0.07%, from 0.07% to 0.08%, from 0.08% to 0.09%, from 0.09% to 0.10%, from 0.10% to 0.11%, from 0.11% to 0.12%, from 0.12% to 0.13%, from 0.13% to 0.14%, from 0.14% to 0.15%, from 0.15% to 0.16%, from 0.16% to 0.17%, from 0.17% to 0.18%, from 0.18% to 0.19%, or from 0.19% to 0.20% of one or more of Mo, Nb, Be, B, Co, Sn, Sr, V, In, Hf, Ag, and Ni. All are expressed in wt.%.

The alloy compositions described herein may further include other minor elements, sometimes referred to as impurities, for example in amounts of 0.05% or below, 0.04% or below, 0.03% or below, 0.02% or below, or 0.01% or below. These impurities may include, but are not limited to Ga, Ca, Bi, Na, Pb, or combinations thereof. Accordingly, Ga, Ca, Bi, Na, or Pb may be present in alloys in amounts of 0.05% or below, 0.04% or below, 0.03% or below, 0.02% or below, or 0.01% or below. The sum of all impurities does not exceed 0.15% (e.g., 0.10%). All expressed in wt.%. The remaining percentage or remainder of any alloy is aluminum.

Aluminum alloy product 210 of FIGs. 2A-2D may include a novel aluminum alloy, as provided herein. The composition and method of making aluminum alloy product 210 may provide for quench insensitivity and improved strength values as compared to aluminum alloy product 110 depicted in FIGs. 1A-1D. FIGS. 2A-2D may exhibit one aspect of aluminum alloy product 210's quench insensitivity. Similar to FIGs. 1A-1D, aluminum alloy product 210 may be quenched at various quenched rates, subjected to corrosion testing, and a corrosion profile provided for each of the different quench rates to illustrate quench sensitivity. Starting at FIG. 2A, aluminum alloy product 210 corresponds to quenching at a rate of 550 °C/s. A quench rate of 550 °C/s may be achieved via water quenching. When quenched at a rapid quench rate of 550 °C/s and subjected to corrosion testing, aluminum alloy product 210 may exhibit pitting corrosion 220, identified by cavities of material loss. Similarly, at FIGs. 2B and 2C, pitting corrosion 220 may also be exhibited when aluminum alloy product 210 is subjected to a quench rate of 350 °C/s and corrosion testing and to a quench rate of 250 °C/s and corrosion testing. In embodiments, a change in corrosion morphology from pitting corrosion 220 to intergranular corrosion 230 may occur at slower quench rates. For example, as provided at FIG. 2D, intergranular corrosion 230 may be exhibited when aluminum alloy product 210 is quenched at 5 °C/s and subjected to corrosion testing. In some cases, aluminum alloy product 210 may exhibit intergranular corrosion 230 upon corrosion testing when the quench rate is at 50 °C/s or less. However, in other cases, little or no intergranular corrosion 230 may be exhibited by aluminum alloy product 210 upon corrosion testing when the quench rate is greater than or about 5 °C/s, such as from 5 °C/s to 25 °C/s, from 25 °C/s to 50 °C/s, from 50 °C/s to 75 °C/s, from 75 °C/s to 100 °C/s, from 100 °C/s to 125 °C/s, from 125 °C/s to 150 °C/s, from 150 °C/s to 175 °C/s, from 175 °C/s to 200 °C/s, from 200 °C/s to 225 °C/s, or from 225 °C/s to 250 °C/s. Slow quench rates, such as quench rates lower than 200 °C/s, lower than 100 °C/s, lower than 50 °C/s, or lower than 25 °C/s, may be achieved by air quenching. Air quenching may include air blasting aluminum alloy product 210 or holding aluminum alloy product 210 at room temperature. Further details regarding quenching are described below.

FIGs. 3A-3D also provide corrosion profiles for a heat-treated aluminum alloy product according to this disclosure at various quench rates. The heat-treated aluminum alloy products may be a quench-insensitive aluminum alloy product and is identified in FIGs. 3A-3D as aluminum alloy product 310. Aluminum alloy product 310 may include a novel aluminum alloy as provided herein. As such, aluminum alloy product 310 may exhibit improved quench insensitivity and corresponding improved strength values, particularly when compared to aluminum alloy product 110 depicted in FIGs. 1A-1D. Aluminum alloy 310 may be quenched according to the quenching methods described herein. Similar to the previously described figures, aluminum alloy 310 may be quenched at a rapid quench rate of 550 °C/s. As depicted at FIG. 3A, aluminum alloy product 310 may exhibit pitting corrosion 320 when quenched at this rapid quench rate and subjected to corrosion testing. Pitting corrosion 320 may also be exhibited at lower quench rates. As shown in FIGs. 3B and 3C, aluminum alloy product 310 may exhibit pitting corrosion 320 upon corrosion testing when quenched at quench rates of 350 °C/s and 250 °C/s. The corrosion morphology may change to intergranular corrosion 130 when the quench rate is slowed below 250 °C/s, such as to 5 °C/s, as illustrated in FIG. 3D. Accordingly, FIGs. 2A-2D and 3A-3D may illustrate one aspect of quench insensitivity exhibited by the novel aluminum alloys provided herein, specifically showing that the corrosion morphology exhibited upon quench testing does not change to intergranular corrosion 130 until quench rates are lower than 250 °C/s.

While FIGs. 1A to 3D may illustrate the type of corrosion formed when a quenched aluminum alloy product is subjected to corrosion testing, FIG. 4 quantifies the extent to which each type of corrosion is exhibited within the product upon testing. FIG. 4 provides an illustrative graph showing a comparison of corrosion depths for regions of corrosion at different quench rates for a quench-sensitive aluminum alloy product versus heat-treated aluminum alloy products made according to this disclosure. FIG. 4 provides three separate graphs positioned side-by-side for ease of comparison of the different aluminum alloy products. FIG. 4 includes graphs 405, 410, and 415, each providing data for a different aluminum alloy product being quenched at various rates. Each of the aluminum alloy products represented in FIG. 4 may have undergone the same processing before being subjected to corrosion testing in accordance with standards ASTM G110, ASTM G129, and/or ASTM G139. These standards provide for aluminum corrosion testing that provides for repeatable measurements of corrosion susceptibility for a particular material. Following ASTM G110 standard, each of the aluminum alloy products used for FIG. 4 may be immersed in sodium chloride and hydrogen peroxide solution. Each of the aluminum alloy products may be immersed for 24 hours and/or 48 hours. Data corresponding to each of the aluminum alloy products were collected and used to generate graphs 405, 410, and 415.

In graph 405, corrosion depth exhibited at various quench rates for a quench-sensitive aluminum alloy product are provided. Graph 405 may correspond to aluminum alloy product 110 and represents an AA7075 aluminum alloy product. As previously discussed with respect to FIGs. 1A-1D, aluminum alloy product 110 may be quench-sensitive and exhibit a change in corrosion morphology from pitting corrosion to intergranular corrosion at higher quench rates. Graph 405 illustrates similar results, showing that pitting corrosion 420 is exhibited at rapid quench rates, such as 550 °C/s and 350 °C/s. However, once the quench rate is reduced to 250 °C/s, the corrosion morphology may change to intergranular corrosion 430. As highlighted by the box in graph 405 labeled "IGC Region", aluminum alloy product 110 may exhibit intergranular corrosion 430 when quenched at any rate at or below 250 °C/s. In some cases, intergranular corrosion may be observed in corrosion tested AA7075 aluminum alloy products processed using quench rates of from about 5 °C/s to about 250 °C/s or from about 5 °C/s to about 350 °C/s, such as from 5 °C/s to 250 °C/s, from 5 °C/s to 260 °C/s, from 5 °C/s to 270 °C/s, from 5 °C/s to 280 °C/s, from 5 °C/s to 290 °C/s, from 5 °C/s to 300 °C/s, from 5 °C/s to 310 °C/s, from 5 °C/s to 320 °C/s, from 5 °C/s to 330 °C/s, from 5 °C/s to 340 °C/s, or from 5 °C/s to 345 °C/s.

Graph 405 also indicates the corrosion depth. Corrosion depth may refer to the extent to which corrosion is exhibited into the bulk of the aluminum alloy from a surface of the aluminum alloy product. In other words, corrosion depth may refer to a depth into the bulk of the aluminum alloy product at which corrosion may be present upon corrosion testing. Graph 405 may include or represent data from multiple quench tests for each quench rate or from multiple locations on the corrosion tested samples. As such, the blocks may correspond to an average corrosion depth observed and standard deviation or error bars may indicate the full range of corrosion depth observed during testing.

As illustrated in graph 405, as the quench rate decreases, the depth of corrosion may increase. Limiting corrosion may be desirable and thus a lower corrosion depth may be desirable as well. As illustrated in graph 405, at a quench rate of 550 °C/s, corrosion 420 may extend to an average depth of about 50 µm into the aluminum alloy product and may correspond to pitting corrosion, for example. When the quench rate is slowed to 350 °C/s, corrosion 420 may extend even further into the aluminum alloy product to an average depth of about 75 µm, and again may correspond to pitting corrosion. When the corrosion morphology changes to intergranular corrosion, the corrosion depth may continue to increase. While the corrosion depth for corrosion 430 may decrease slightly when the aluminum alloy product is quenched at a rate of 150 °C/s, this point includes large error bars where the maximum corrosion depth is quite large. The average corrosion depth of corrosion 430 for quench rates of from 5 °C/s to 250 °C/s may still be greater than the corrosion depth at rapid quench rates, such as 550 °C/s. Even at a slow quench rate of 5 °C/s, corrosion may extend to a corrosion depth of about 85 µm.

Graphs 410 and 415 illustrate corrosion depths observed for additional aluminum alloy products according to the present disclosure. The aluminum alloy products for which data are shown in graphs 410 and 415 may be heat-treated aluminum alloy products. The heat-treated aluminum alloy product may be a quench-insensitive aluminum alloy product such as aluminum alloy products 210 and 310. The heat-treated aluminum alloy product observed may be an aluminum alloy product made according to the methods and compositions described herein. For example, such aluminum alloy products may be made from an aluminum alloy having the following elemental composition as provided in Table 5.

**Table 5.**

| Element | Aluminum alloy 4A Weight Percentage (wt.%) (not according to the invention) | Aluminum alloy 4B Weight Percentage (wt.%) |
|---|---|---|
| Zn | 9.00 | 9.16 |
| Cu | 1.18 | 1.18 |
| Mg | 2.29 | 2.29 |
| Fe | 0.20 | 0.23 |
| Si | 0.10 | 0.10 |
| Zr | 0.11 | 0.11 |
| Mn | 0.04 | 0.04 |
| Cr | 0.10 | 0.04 |
| Ti | n/a | 0.01 |
| Al | Remainder | Remainder |

As illustrated in graph 410, when the aluminum alloy product 4A is quenched and subjected to corrosion testing, corrosion 420 may be observed for most of the quench rates. For example, pitting corrosion may be exhibited even at slow quench rates of 50 °C/s or less. In the data obtained, when quench rates are slowed to 5 °C/s, aluminum alloy product 4A exhibits intergranular corrosion 430 (IGC). Moreover, the corrosion exhibited by aluminum alloy product 4A for which data are shown in graph 410, regardless of the type of corrosion, generally has an overall reduced corrosion depth when compared with the quench-sensitive aluminum alloy product of graph 405. Even at the slowest quench rate of 5 °C/s, a lower corrosion depth is observed. While the corrosion depth may increase somewhat as the quench rate decreases, the rate of increase in corrosion depth over the quench rates may be minimal. For example, the corrosion depth of corrosion 420 shown in graph 410 at a quench rate of 550 °C/s may be about 40 µm, while the corrosion depth at a quench rate of 5 °C/s is only slightly more, at about 50 µm. Overall, the corrosion depth shown in graph 410 is relatively constant when compared to the quench-sensitive aluminum alloy product of graph 405. Additionally, as indicated by the standard deviation bars, corrosion depth may also be relatively constant across multiple runs of the same test. The lack of deviation between different trial runs of the same tests (i.e., multiple quenches at the same quench rate) may further show the aluminum alloy product's insensitivity to quenching by indicating that changes in operating conditions may have minimal effect on corrosion susceptibility.

Graph 415 may indicate similar quenching insensitivity for another aluminum alloy product 4B as described herein. Similar to the aluminum alloy product 4A for which data are shown in graph 410, corrosion morphology for the aluminum alloy product represented by graph 415 may not change from pitting corrosion to intergranular corrosion until a quench rate of or below 5 °C/s. Unexpectedly, corrosion depths may decrease in some cases as the quench rate decreases. This result is unexpected when comparing corrosion depth trends with respect to quench rates on graphs 405 and 410 which indicate an increase in corrosion depth with decreasing quench rates. In graph 415, rates from 50 °C/s to 250 °C/s may represent that pitting corrosion is the primary corrosion 420 extending to corrosion depths of about 25 µm or less. As illustrated by graphs 410 and 415, when quench rates of from 5 °C/s to 550 °C/s are used, corrosion depth upon corrosion testing may be from 0 µm to 300 µm, 5 µm to 300 µm, 0 µm to 200 µm, from 5 µm to 100 µm, or from 10 µm to 80 µm. For example, when the quench rate is 125 °C/s the corrosion depth may be from 5 µm to 150 µm or from 25 µm to 50 µm.

As discussed previously, quench sensitivity may impact the properties of an aluminum alloy product, specifically the strength values. Exemplary strength characteristics may include yield strength, tensile strength, grain elongation, and strain ratio. FIGs. 5 to 8 provide illustrative graphs depicting comparison data between a quench-sensitive aluminum alloy product and heat-treated aluminum alloy products made according to methods and techniques provided herein. The quench-sensitive aluminum alloy product is represented by the data labeled "C" (black square) on the graphs in FIGs. 5 to 8. **In** some embodiments, aluminum alloy product C may include a 7xxx series aluminum alloy product made in accordance with conventional methods and techniques. For example, aluminum alloy product C may correspond to an AA7075 aluminum alloy product (similar to aluminum alloy product 110). Data labeled "5A" (red circle) and "5B" (blue triangle) on the graphs in FIGs. 5 to 8 represent heat-treated aluminum alloy products that are quench-insensitive aluminum alloy products. Aluminum alloy products 5A and 5B may be made from aluminum alloys having the following elemental compositions as provided in Table 6.

**Table 6.**

| Element | Aluminum alloy 5A Weight Percentage (wt.%) (not according to the invention) | Aluminum alloy 5B Weight Percentage (wt.%) |
|---|---|---|
| Zn | 9.00 | 9.16 |
| Cu | 1.18 | 1.18 |
| Mg | 2.29 | 2.29 |
| Fe | 0.20 | 0.23 |
| Si | 0.10 | 0.10 |
| Zr | 0.11 | 0.12 |
| Mn | 0.04 | 0.04 |
| Cr | 0.10 | 0.04 |
| Ti | n/a | 0.01 |
| Al | Remainder | Remainder |

Each of the aluminum alloy products 5A, 5B, and C may be prepared prior to being subjected to the same mechanical testing procedure. To prepare aluminum alloy products 5A, 5B, and C, the aluminum alloy products may be solutionized to a first temperature of 480 °C. The aluminum alloy products may be maintained or held at the first temperature for 5 minutes before being quenched in water baths maintained at temperatures of 25 °C, 55 °C, 65 °C, 75 °C, 85 °C to achieve quench rates of 550 °C/s, 350 °C/s, 250 °C/s, 150 °C/s, and 50 °C/s, respectively. To achieve the quench rate of 5 °C/s, the aluminum alloy products may be air quenched. After quenching, the aluminum alloy products may be subjected to a one step aging process. An exemplary aging process may include a T6 or T7 temper or precipitation hardening. For the graphs in FIGs. 5 to 8, the aluminum alloy products may be subjected to an aging process in which the products may be reheated to a temperature of 125 °C for 25 hours. After being subjected to this aging process, the aluminum alloy products may be subjected to mechanical testing, corrosion testing in accordance with ASTM G110, stress corrosion evaluation in accordance with ASTM G129, and/or stress corrosion evaluation in accordance with ASTM G139. The following FIGs. 5-9, 10A-10C, and 11A-11C provide data gathered from testing of aluminum alloy products 5A, 5B, and C prepared and conducted in accordance with the above discussed processes.

FIG. 5 provides graph 500 illustrating a comparison of yield strengths exhibited by aluminum alloy products 5A, 5B, and C. Yield strength, also known as yield stress, is a material property that defines the stress at which a material begins to plastically deform. Plastic deformation is the permanent distortion of a product under stress such as elongation, compression, buckling, bending, or twisting. Yield strength may be an important component when characterizing the strength of an aluminum alloy product.

As shown on graph 500, aluminum alloy products 5A and 5B made from the quench insensitive 7xxx series aluminum alloy compositions, as provided above and made according to the techniques provided herein, may exhibit superior yield strength when compared to aluminum alloy product C. For example, aluminum alloy products 5A and 5B may exhibit yield strengths from 400 MPa to 600 MPa. Specifically, aluminum alloy products 5A and 5B may exhibit yield strengths from 500 MPa to 650 MPa at quench rates from 50 °C/s to 550 °C/s. For example, aluminum alloy products 5A and 5B may exhibit a yield strength of from 560 MPa to 580 MPa when the quench rate is 125 °C/s. In some embodiments, quench insensitive aluminum alloy products may exhibit yield strengths from about 550 MPa to about 600 MPa at quench rates from 50 °C/s to 550 °C/s or yield strengths from about 525 MPa to about 600 MPa at quench rates from 350 °C/s to 550 °C/s. For example, at a quench rate of 550 °C/s, aluminum alloy products 5A and 5B may exhibit a yield strength of about 572 MPa and about 579 MPa, respectively. In comparison, aluminum alloy product C may exhibit a yield strength of about 532 MPa at a quench rate of 550 °C/s. At quench rates of 350 °C/s and 50 °C/s, aluminum alloy product 5A may exhibit yield strengths of about 572 MPa and 553 MPa, respectively, and aluminum alloy product 5B may exhibit yield strengths of about 575 MPa and 569 MPa, respectively. In comparison, aluminum alloy product C may exhibit yield strengths of about 524 and 509 at quench rates of 350 °C/s and 50 °C/s, respectively.

The improved yield strength of aluminum alloy products 5A and 5B may be even more evident at low quench rates, such as the quench rate of 5 °C/s. At a quench rate of 5 °C/s, aluminum alloy products 5A and 5B exhibit yield strengths of about 439 MPa and 489 MPa, which may be almost 100 MPa higher than the yield strength of aluminum alloy product C at a quench rate of 5 °C/s. At 5 °C/s, aluminum alloy product C exhibits a yield strength of about 347 MPa. Advantageously, aluminum alloy products 5A and 5B exhibit a drop in yield strength of less than 25% when the quench rate is slowed from 550 °C/s to 5 °C/s. In comparison, aluminum alloy product C exhibits a drop of over 25%, such as for example 35%, when the quench rate is slowed from 550 °C/s to 5 °C/s.

FIG. 6 provides graph 600 illustrating a comparison of ultimate tensile strength exhibited by aluminum alloy products 5A, 5B, and C. Ultimate tensile strength (UTS) may correspond to the capacity of a material to withstand elongation loads. In contrast to a stress test in which a force exerted on a material tends to reduce the size of the material, tensile strength stress tests the ability of the material to withstand elongation. Ultimate tensile strength can be measured by the maximum stress that a material can withstand while being stretched or pulled before breaking.

Similar to yield strength, aluminum alloy products 5A and 5B may exhibit superior ultimate tensile strength over various quench rates when compared with aluminum alloy product C. As shown on graph 600, aluminum alloy products 5A and 5B exhibit ultimate tensile strengths (also referred to herein as tensile strengths) from 500 MPa to 650 MPa at quench rates from 5 °C/s to 550 °C/s. For example, aluminum alloy products 5A and 5B may exhibit an ultimate tensile strength of from 605 MPa to 615 MPa when the quench rate is 125 °C/s. In some embodiments, quench insensitive aluminum alloy products may exhibit tensile strengths from 585 MPa to 625 MPa at quench rates from 50 °C/s to 550 °C/s. For example, at a quench rate of 550 °C/s, aluminum alloy products A and B exhibit tensile strengths of about 614 MPa and about 618 MPa, respectively. In comparison, aluminum alloy product C exhibits a tensile strength of about 584 MPa at a quench rate of 550 °C/s. At quench rates of 350 °C/s and 50 °C/s, aluminum alloy product 5A exhibits tensile strengths of about 614 MPa and about 593 MPa, respectively, and aluminum alloy product 5B exhibits tensile strengths of about 618 MPa and about 605 MPa, respectively. In comparison, aluminum alloy product C exhibits tensile strengths of about 578 MPa and about 566 MPa at quench rates of 350 °C/s and 50 °C/s, respectively.

Even at slow quench rates, such as 5 °C/s, aluminum alloy products 5A and 5B exhibit higher tensile strengths as compared to aluminum alloy product C. For example, at a quench rate of 5 °C/s, quench insensitive aluminum alloy products may exhibit tensile strengths of from about 475 MPa to about 550 MPa. As illustrated in FIG. 6, the tensile strength at 5 °C/s for aluminum alloy products 5A and 5B are about 507 MPa and about 544 MPa, respectively. In comparison, aluminum alloy product C exhibits a tensile strength of about 458 MPa when quenched at a rate of 5 °C/s.

Turning now to FIG. 7, total elongation (TE) of aluminum alloy products 5A, 5B, and C when subjected to stress may be illustrated. Total elongation, expressed as a percentage of change over a fixed gauge, may correspond to the percentage by which a material can be stretched before it breaks. In some embodiments, total elongation may be a rough indicator of formability of aluminum alloy products.

As illustrated by graph 700, aluminum alloy products 5A and 5B may exhibit a total elongation from 10.00% to 15.00% for quench rates from 5 °C/s to 550 °C/s. For example, at rapid quench rates, such as 550 °C/s, aluminum alloy products 5A and 5B exhibit a total elongation of about 14.70% and about 14.31%, respectively. As the quench rate is slowed to 350 °C/s, 50 °C/s, and 5 °C/s, aluminum alloy product 5A exhibits a total elongation of about 15.10%, about 13.29%, and about 10.46%, respectively. Similarly, aluminum alloy product 5B exhibits a total elongation of 14.48%, 13.65%, and 10.15% when the quench rate is slowed to 350 °C/s, 50 °C/s, and 5 °C/s, respectively. When the quench rate is 125 °C/s, aluminum alloy products 5A and 5B may exhibit a total elongation of from 13.80% to 14.20%. In some cases, quench insensitive aluminum alloy products may exhibit a uniform elongation of from 7.50% to 10.50%. For example, aluminum alloy products 5A and 5B may exhibit a uniform elongation of from 9.00% to 9.60% when the quench rate is 125 °C/s.

As illustrated in FIG. 7, aluminum alloy product C may exhibit a total elongation from 14.09% to 15.25% for quench rates from 5 °C/s to 550 °C/s. For example, aluminum alloy product C may exhibit a total elongation of more than 15.00% at a quench rate of 550 °C/s. As the quench rate is slowed to 350 °C/s, 50 °C/s, and 5 °C/s, aluminum alloy product C may exhibit a total elongation of about 14.60%, about 14.31%, and about 14.09%, respectively. Uniform elongation may correspond to the elongation of a material at a maximum load until necking occurs. In some cases, uniform elongation may represent a material's ductility or formability in uniaxial deformation.

FIG. 8 provides graph 800 illustrating a comparison of strain ratio exhibited by aluminum alloy products 5A, 5B, and C. Strain ratio may be a useful measure of the stress corrosion cracking susceptibility. For example, the lower the strain ratio, the greater the stress corrosion cracking susceptibility may be for an aluminum alloy product. As illustrated by graph 800, the strain ratios exhibited by aluminum alloy products 5A and 5B may be consistently higher than the strain ratios exhibited by aluminum alloy product C. Even at slow quench rates, such as 5 °C/s, where intergranular corrosion may be observed, the strain ratios exhibited by aluminum alloy products 5A and 5B may be higher than the strain ratios exhibited by aluminum alloy product C.

In embodiments, quench insensitive aluminum alloy products may exhibit a strain ratio from 0.3 to 1.0 for quench rates from 5 °C/s to 550 °C/s. In other embodiments, the strain ratios may be from 0.5 to 1.0 when quench insensitive aluminum alloy products are quenched at rates from 250 °C/s to 500 °C/s. When the quench rate is 125 °C/s, aluminum alloy products 5A and 5 B may exhibit a strain ratio of 0.375 to 0.425. For example, when aluminum alloy products 5A and 5B are quenched at a rapid rate of 550 °C/s, the strain ratio may be from 0.5 to 1.0. As illustrated by graph 800, for all of the quench rates tested, aluminum alloy products 5A and 5B may exhibit a strain ratio above 0.3. In comparison, strain ratios exhibited by aluminum alloy product C may be below 0.3 across all of the quench rates tested. This may indicate that aluminum alloy product C is more susceptible to stress corrosion cracking than aluminum alloy products 5A and 5B.

FIG. 9 provides graph 900, which illustrates a comparison of precipitate-free zones exhibited by aluminum alloy products 5A, 5B, and C. During an aging process, precipitation may be exhibited when solutes and other hardening compounds precipitate out of the aluminum alloy solution. Zones or pockets in which little or no precipitation is exhibited may be referred to as precipitate-free zones. Precipitate-free zones may be exhibited because precipitates, such as solutes, nucleate heterogeneously on vacancies. A grain boundary may be a sink for vacancies so regions adjacent to boundaries may be unable to nucleate the precipitate, even though the alloy solution may be supersaturated with solute. Precipitate-free zones may be undesirable because they may act as regions of weakness. For example, precipitate-free zones may be more susceptible to corrosive attack than other points within the aluminum alloy. Accordingly, reducing the amount and width of precipitate-free zones may be desirable to improve the strength and corrosion susceptibility of an aluminum alloy product.

As illustrated by graph 900, the width of precipitate-free zones formed during an aging process may increase as quench rate decreases. Aluminum alloy product C may exhibit larger precipitate-free zones during quenching when compared with aluminum alloy products 5A and 5B. For example, at rapid quenching rates, such as 550 °C/s, aluminum alloy product C may exhibit precipitate-free zones having an average width of about 45 nm. In comparison, at a quench rate of 550 °C/s, aluminum alloy products 5A and 5B may exhibit precipitate-free zones having an average width of about 35 nm and 32 nm, respectively. Even at slow quench rates, aluminum alloy product C may exhibit larger precipitate-free zones than aluminum alloy products 5A and 5B. For example, at 5 °C/s, aluminum alloy product C may exhibit precipitate-free zones having an average width of about 200 nm, whereas aluminum alloy products 5A and 5B may exhibit precipitate-free zones having an average width of about 90 nm and 150 nm, respectively.

FIGs. 10A-10C and 11A-11C depict images corresponding to the aluminum alloy products 5A and C illustrated in graph 900 of FIG. 9. For example, the images provided in FIGs. 10A, 10B, and 10C may be taken using scanning transmission electron microscopy (STEM) methods depicting precipitate-free zones 1010 which may correspond to one or more data points on graph 900. That is, the widths or measurements of precipitate-free zones 1010 provided in FIGs. 10A-11C may be used in graph 900.

FIGs. 10A-10C correspond to aluminum alloy product C. FIG. 10A depicts precipitate-free zones 1010 exhibited after aluminum alloy product C is quenched at a rate of 550 °C/s. FIGs. 10B and 10C depict precipitate-free zones 1010 exhibited after aluminum alloy product C is quenched at rates of 150 °C/s and 5 °C/s. As shown, precipitate-free zones 1010 may increase in size (e.g., width) as the quench rate is slowed. FIGs. 11A, 11B, and 11C may provide similar images taken using STEM methods depicting precipitate-free zones 1010 exhibited by aluminum alloy product 5A. FIG. 11A depicts precipitate-free zones 1010 exhibited after aluminum alloy product 5A is quenched at 550 °C/s. Similarly, FIGs. 11B and 11C depict precipitate-free zones 1110 exhibited after aluminum alloy product 5A is quenched at 150 °C/s and 5 °C/s, respectively. While the precipitate-free zones 1110 of aluminum alloy product 5A may become larger as the quench rate is slowed, the width of the precipitate-free zones may be less than that of precipitate-free zones 1010 exhibited by aluminum alloy product C quenched at the same rate. This is also depicted by the data provided in graph 900 of FIG. 9. For example, as illustrated in graph 900, when aluminum alloy product 5A is quenched from 0.5 °C/s to 125 °C/s, then the precipitate free zone widths may range from 10 nm to 110 nm. Specifically, when aluminum alloy product 5A is quenched at 125 °C/s, then aluminum alloy product 5A may exhibit precipitate free zone widths from 10 nm to 13 nm.

It should be noted that while the above discussed improved corrosion resistance and mechanical properties are provided with reference to discrete quench rates, this is not meant to be limiting. Similar properties may be exhibited for a range of quench rates. The improved corrosion resistance and mechanical properties described with reference to FIGs. 1 to 9 may be exhibited for the aluminum alloy products provided here in when the quench rate is from 0.5 °C/s to 125 °C/s. For example, the quench rate may range from 5 °C/s to 125 °C/s, 10 °C/s to 125 °C/s, 15 °C/s to 125 °C/s, 20 °C/s to 125 °C/s, 25 °C/s to 125 °C/s, 30 °C/s to 125 °C/s, 35 °C/s to 125 °C/s, 40 °C/s to 125 °C/s, 45 °C/s to 125 °C/s, 50 °C/s to 125 °C/s, 55 °C/s to 125 °C/s, 60 °C/s to 125 °C/s, 65 °C/s to 125 °C/s, 70 °C/s to 125 °C/s, 75 °C/s to 125 °C/s, 80 °C/s to 125 °C/s, 85 °C/s to 125 °C/s, 90 °C/s to 125 °C/s, 95 °C/s to 125 °C/s, 100 °C/s to 125 °C/s, 105 °C/s to 125 °C/s, 110 °C/s to 125 °C/s, 115 °C/s to 125 °C/s, 120 °C/s to 125 °C/s, 5 °C/s to 120 °C/s, 10 °C/s to 120 °C/s, 15 °C/s to 120 °C/s, 20 °C/s to 120 °C/s, 25 °C/s to 120 °C/s, 30 °C/s to 120 °C/s, 35 °C/s to 120 °C/s, 40 °C/s to 120 °C/s, 45 °C/s to 120 °C/s, 50 °C/s to 120 °C/s, 55 °C/s to 120 °C/s, 60 °C/s to 120 °C/s, 65 °C/s to 120 °C/s, 70 °C/s to 120 °C/s, 75 °C/s to 120 °C/s, 80 °C/s to 120 °C/s, 85 °C/s to 120 °C/s, 90 °C/s to 120 °C/s, 95 °C/s to 120 °C/s, 100 °C/s to 120 °C/s, 105 °C/s to 120 °C/s, 110 °C/s to 120 °C/s, 115 °C/s to 120 °C/s, 5 °C/s to 115 °C/s, 10 °C/s to 115 °C/s, 15 °C/s to 115 °C/s, 20 °C/s to 115 °C/s, 25 °C/s to 115 °C/s, 30 °C/s to 115 °C/s, 35 °C/s to 115 °C/s, 40 °C/s to 115 °C/s, 45 °C/s to 115 °C/s, 50 °C/s to 115 °C/s, 55 °C/s to 115 °C/s, 60 °C/s to 115 °C/s, 65 °C/s to 115 °C/s, 70 °C/s to 115 °C/s, 75 °C/s to 115 °C/s, 80 °C/s to 115 °C/s, 85 °C/s to 115 °C/s, 90 °C/s to 115 °C/s, 95 °C/s to 115 °C/s, 100 °C/s to 115 °C/s, 105 °C/s to 115 °C/s, 110 °C/s to 115 °C/s, 5 °C/s to 110 °C/s, 10 °C/s to 110 °C/s, 15 °C/s to 110 °C/s, 20 °C/s to 110 °C/s, 25 °C/s to 110 °C/s, 30 °C/s to 110 °C/s, 35 °C/s to 110 °C/s, 40 °C/s to 110 °C/s, 45 °C/s to 110 °C/s, 50 °C/s to 110 °C/s, 55 °C/s to 110 °C/s, 60 °C/s to 110 °C/s, 65 °C/s to 110 °C/s, 70 °C/s to 110 °C/s, 75 °C/s to 110 °C/s, 80 °C/s to 110 °C/s, 85 °C/s to 110 °C/s, 90 °C/s to 110 °C/s, 95 °C/s to 110 °C/s, 100 °C/s to 110 °C/s, 105 °C/s to 110 °C/s, 5 °C/s to 105 °C/s, 10 °C/s to 105 °C/s, 15 °C/s to 105 °C/s, 20 °C/s to 105 °C/s, 25 °C/s to 105 °C/s, 30 °C/s to 105 °C/s, 35 °C/s to 105 °C/s, 40 °C/s to 105 °C/s, 45 °C/s to 105 °C/s, 50 °C/s to 105 °C/s, 55 °C/s to 105 °C/s, 60 °C/s to 105 °C/s, 65 °C/s to 105 °C/s, 70 °C/s to 105 °C/s, 75 °C/s to 105 °C/s, 80 °C/s to 105 °C/s, 85 °C/s to 105 °C/s, 90 °C/s to 105 °C/s, 95 °C/s to 105 °C/s, 100 °C/s to 105 °C/s, 5 °C/s to 100 °C/s, 10 °C/s to 100 °C/s, 15 °C/s to 100 °C/s, 20 °C/s to 100 °C/s, 25 °C/s to 100 °C/s, 30 °C/s to 100 °C/s, 35 °C/s to 100 °C/s, 40 °C/s to 100 °C/s, 45 °C/s to 100 °C/s, 50 °C/s to 100 °C/s, 55 °C/s to 100 °C/s, 60 °C/s to 100 °C/s, 65 °C/s to 100 °C/s, 70 °C/s to 100 °C/s, 75 °C/s to 100 °C/s, 80 °C/s to 100 °C/s, 85 °C/s to 100 °C/s, 90 °C/s to 100 °C/s, 95 °C/s to 100 °C/s, 5 °C/s to 105 °C/s, 10 °C/s to 105 °C/s, 15 °C/s to 105 °C/s, 20 °C/s to 105 °C/s, 25 °C/s to 105 °C/s, 30 °C/s to 105 °C/s, 35 °C/s to 105 °C/s, 40 °C/s to 105 °C/s, 45 °C/s to 105 °C/s, 50 °C/s to 105 °C/s, 55 °C/s to 105 °C/s, 60 °C/s to 105 °C/s, 65 °C/s to 105 °C/s, 70 °C/s to 105 °C/s, 75 °C/s to 105 °C/s, 80 °C/s to 105 °C/s, 85 °C/s to 105 °C/s, 90 °C/s to 105 °C/s, 95 °C/s to 105 °C/s, 100 °C/s to 105 °C/s, 5 °C/s to 95 °C/s, 10 °C/s to 95 °C/s, 15 °C/s to 95 °C/s, 20 °C/s to 95 °C/s, 25 °C/s to 95 °C/s, 30 °C/s to 95 °C/s, 35 °C/s to 95 °C/s, 40 °C/s to 95 °C/s, 45 °C/s to 95 °C/s, 50 °C/s to 95 °C/s, 55 °C/s to 95 °C/s, 60 °C/s to 95 °C/s, 65 °C/s to 95 °C/s, 70 °C/s to 95 °C/s, 75 °C/s to 95 °C/s, 80 °C/s to 95 °C/s, 85 °C/s to 95 °C/s, 90 °C/s to 95 °C/s, 5 °C/s to 90 °C/s, 10 °C/s to 90 °C/s, 15 °C/s to 90 °C/s, 20 °C/s to 90 °C/s, 25 °C/s to 90 °C/s, 30 °C/s to 90 °C/s, 35 °C/s to 90 °C/s, 40 °C/s to 90 °C/s, 45 °C/s to 90 °C/s, 50 °C/s to 90 °C/s, 55 °C/s to 90 °C/s, 60 °C/s to 90 °C/s, 65 °C/s to 90 °C/s, 70 °C/s to 90 °C/s, 75 °C/s to 90 °C/s, 80 °C/s to 90 °C/s, 85 °C/s to 90 °C/s, 5 °C/s to 85 °C/s, 10 °C/s to 85 °C/s, 15 °C/s to 85 °C/s, 20 °C/s to 85 °C/s, 25 °C/s to 85 °C/s, 30 °C/s to 85 °C/s, 35 °C/s to 85 °C/s, 40 °C/s to 85 °C/s, 45 °C/s to 85 °C/s, 50 °C/s to 85 °C/s, 55 °C/s to 85 °C/s, 60 °C/s to 85 °C/s, 65 °C/s to 85 °C/s, 70 °C/s to 85 °C/s, 75 °C/s to 85 °C/s, 80 °C/s to 85 °C/s, 5 °C/s to 80 °C/s, 10 °C/s to 80 °C/s, 15 °C/s to 80 °C/s, 20 °C/s to 80 °C/s, 25 °C/s to 80 °C/s, 30 °C/s to 80 °C/s, 35 °C/s to 80 °C/s, 40 °C/s to 80 °C/s, 45 °C/s to 80 °C/s, 50 °C/s to 80 °C/s, 55 °C/s to 80 °C/s, 60 °C/s to 80 °C/s, 65 °C/s to 80 °C/s, 70 °C/s to 80 °C/s, 75 °C/s to 80 °C/s, 5 °C/s to 75 °C/s, 10 °C/s to 75 °C/s, 15 °C/s to 75 °C/s, 20 °C/s to 75 °C/s, 25 °C/s to 75 °C/s, 30 °C/s to 75 °C/s, 35 °C/s to 75 °C/s, 40 °C/s to 75 °C/s, 45 °C/s to 75 °C/s, 50 °C/s to 75 °C/s, 55 °C/s to 75 °C/s, 60 °C/s to 75 °C/s, 65 °C/s to 75 °C/s, 70 °C/s to 75 °C/s, 5 °C/s to 70 °C/s, 10 °C/s to 70 °C/s, 15 °C/s to 70 °C/s, 20 °C/s to 70 °C/s, 25 °C/s to 70 °C/s, 30 °C/s to 70 °C/s, 35 °C/s to 70 °C/s, 40 °C/s to 70 °C/s, 45 °C/s to 70 °C/s, 50 °C/s to 70 °C/s, 55 °C/s to 70 °C/s, 60 °C/s to 70 °C/s, 65 °C/s to 70 °C/s, 5 °C/s to 65 °C/s, 10 °C/s to 65 °C/s, 15 °C/s to 65 °C/s, 20 °C/s to 65 °C/s, 25 °C/s to 65 °C/s, 30 °C/s to 65 °C/s, 35 °C/s to 65 °C/s, 40 °C/s to 65 °C/s, 45 °C/s to 65 °C/s, 50 °C/s to 65 °C/s, 55 °C/s to 65 °C/s, 60 °C/s to 65 °C/s, 5 °C/s to 60 °C/s, 10 °C/s to 60 °C/s, 15 °C/s to 60 °C/s, 20 °C/s to 60 °C/s, 25 °C/s to 60 °C/s, 30 °C/s to 60 °C/s, 35 °C/s to 60 °C/s, 40 °C/s to 60 °C/s, 45 °C/s to 60 °C/s, 50 °C/s to 60 °C/s, 55 °C/s to 60 °C/s, 5 °C/s to 55 °C/s, 10 °C/s to 55 °C/s, 15 °C/s to 55 °C/s, 20 °C/s to 55 °C/s, 25 °C/s to 55 °C/s, 30 °C/s to 55 °C/s, 35 °C/s to 55 °C/s, 40 °C/s to 55 °C/s, 45 °C/s to 55 °C/s, 50 °C/s to 55 °C/s, 5 °C/s to 50 °C/s, 10 °C/s to 50 °C/s, 15 °C/s to 50 °C/s, 20 °C/s to 50 °C/s, 25 °C/s to 50 °C/s, 30 °C/s to 50 °C/s, 35 °C/s to 50 °C/s, 40 °C/s to 50 °C/s, 45 °C/s to 50 °C/s, 5 °C/s to 45 °C/s, 10 °C/s to 45 °C/s, 15 °C/s to 45 °C/s, 20 °C/s to 45 °C/s, 25 °C/s to 45 °C/s, 30 °C/s to 45 °C/s, 35 °C/s to 45 °C/s, 40 °C/s to 45 °C/s, 5 °C/s to 40 °C/s, 10 °C/s to 40 °C/s, 15 °C/s to 40 °C/s, 20 °C/s to 40 °C/s, 25 °C/s to 40 °C/s, 30 °C/s to 40 °C/s, 35 °C/s to 40 °C/s, 5 °C/s to 35 °C/s, 10 °C/s to 35 °C/s, 15 °C/s to 35 °C/s, 20 °C/s to 35 °C/s, 25 °C/s to 35 °C/s, 30 °C/s to 35 °C/s, 5 °C/s to 30 °C/s, 10 °C/s to 30 °C/s, 15 °C/s to 30 °C/s, 20 °C/s to 30 °C/s, 25 °C/s to 30 °C/s, 5 °C/s to 25 °C/s, 10 °C/s to 25 °C/s, 15 °C/s to 25 °C/s, 20 °C/s to 25 °C/s, 5 °C/s to 20 °C/s, 10 °C/s to 20 °C/s, 15 °C/s to 20 °C/s, 5 °C/s to 15 °C/s, 10 °C/s to 15 °C/s, or 5 °C/s to 10 °C/s.

FIG. 12 provides an overview of a method 1200 of making a quench-insensitive aluminum alloy product. At block 1205, an aluminum alloy product is subjected to one or more rolling or forming processes. The one or more rolling or forming processes may include a hot rolling process at block 1207, a cold rolling process at block 1209, or both. Optionally, the heat-treated aluminum alloy product may be cold rolled to a final gauge thickness. The final gauge thickness may be from 0.2 mm to 10.0 mm (e.g., 2.0 mm). For example, the heat-treated aluminum alloy product may be cold rolled to a final gauge thickness of 0.2 mm, 0.3 mm, 0.4 mm, 0.5 mm, 0.6 mm, 0.7 mm, 0.8 mm, 0.9 mm, 1.0 mm, 1.1 mm, 1.2 mm, 1.3 mm, 1.4 mm, 1.5 mm, 1.6 mm, 1.7 mm, 1.8 mm, 1.9 mm, 2.0 mm, 2.1 mm, 2.2 mm, 2.3 mm, 2.4 mm, 2.5 mm, 2.6 mm, 2.7 mm, 2.8 mm, 2.9 mm, 3.0 mm, 3.1 mm, 3.2 mm, 3.3 mm, 3.4 mm, 3.5 mm, 3.6 mm, 3.7 mm, 3.8 mm, 3.9 mm, 4.0 mm, 4.1 mm, 4.2 mm, 4.3 mm, 4.4 mm, 4.5 mm, 4.6 mm, 4.7 mm, 4.8 mm, 4.9 mm, 5.0 mm, 5.1 mm, 5.2 mm, 5.3 mm, 5.4 mm, 5.5 mm, 5.6 mm, 5.7 mm, 5.8 mm, 5.9 mm, 6.0 mm, 6.1 mm, 6.2 mm, 6.3 mm, 6.4 mm, 6.5 mm, 6.6 mm, 6.7 mm, 6.8 mm, 6.9 mm, 7.0 mm, 7.1 mm, 7.2 mm, 7.3 mm, 7.4 mm, 7.5 mm, 7.6 mm, 7.7 mm, 7.8 mm, 7.9 mm, 8.0 mm, 8.1 mm, 8.2 mm, 8.3 mm, 8.4 mm, 8.5 mm, 8.6 mm, 8.7 mm, 8.8 mm, 8.9 mm, 9.0 mm, 9.1 mm, 9.2 mm, 9.3 mm, 9.4 mm, 9.5 mm, 9.6 mm, 9.7 mm, 9.8 mm, 9.9 mm, or 10.0 mm. The cold rolling may be performed to result in the heat-treated aluminum alloy product having a final gauge thickness that represents an overall gauge reduction by 20%, 50%, 75%, or 85%.

At block 1210, the rolled aluminum alloy product is heated. The rolled aluminum alloy product may be a quench-insensitive aluminum alloy product. In embodiments, the rolled aluminum alloy product may include an aluminum alloy having an elemental composition according to those provided in Tables 5 and 6. The rolled aluminum alloy product includes a 7xxx series aluminum alloy as defined in the claims. In embodiments, the rolled aluminum alloy product may be a slab, strip, plate, shate, or sheet. Optionally, ingots and/or billets may be used with method 1200.

The rolled aluminum alloy product is heated to a first temperature at block 1210. The rolled aluminum alloy product may be heated during a heat treatment process. In some embodiments, the heat treatment process may be a solutionizing heat treatment process. During heating, the rolled aluminum alloy product is heated to a first temperature of at least 400 °C to 525 °C (e.g., at least 425 °C, at least 450 °C, at least 460 °C, or at least 465 °C). In some cases, the first temperature may range from 400 °C to 525 °C, 425 °C to 510 °C, 450 °C to 510 °C, 450 °C to 500 °C, 450 °C to 480 °C, or 450 °C to 475 °C. The first temperature may be a solutionizing temperature in some embodiments.

During heating the rolled aluminum alloy product, the heating rate to the first temperature may be 70 °C/hour or less, 60 °C/hour or less, or 50 °C/hour or less.

In embodiments, the heat treatment process may be or include a hot rolling process. The hot rolling process may include a hot reversing mill operation and/or a hot tandem mill operation. The hot rolling process may be performed at a temperature ranging from about 250 °C to about 550 °C (e.g., from about 300 °C to about 500 °C or from about 350 °C to about 450 °C). In the hot rolling process, the rolled aluminum alloy product may be hot rolled to a 12 mm thick gauge or less (e.g., from 3 mm to 8 mm thick gauge). For example, the rolled aluminum alloy product may be hot rolled to a 11 mm thick gauge or less, 10 mm thick gauge or less, 9 mm thick gauge or less, 8 mm thick gauge or less, 7 mm thick gauge or less, 6 mm thick gauge or less, 5 mm thick gauge or less, 4 mm thick gauge or less, or 3 mm thick gauge or less. In some embodiments, the hot rolling process may occur at a different point during method 1200. For example, the hot rolling process may occur after a forming or after a quenching step.

The rolled aluminum alloy product may be maintained at the first temperature, or within 10 °C of the first temperature, for a time duration of from 30 seconds to 30 minutes at block 1220. In some cases, the time duration is from 15 seconds to 30 minutes, 15 seconds to 5 minutes15 seconds to 30 seconds, 30 seconds to 6 hours, 30 seconds to 3 hours, 30 seconds to 1 hour, 30 seconds to 30 minutes, 30 seconds to 5 minutes, 30 seconds to 1 minute, 1 minute to 30 minutes, 5 minutes to 30 minutes. Optionally, the rolled aluminum alloy product may be maintained within 5 °C of the first temperature, or within 1 °C of the first temperature for the specified time duration.

At the end of the heat treatment process, the rolled aluminum alloy product may optionally be subjected to one or more forming processes at block 1230. For example, at block 1230, the rolled aluminum alloy product may be subjected to a hot forming process. In some embodiments, the rolled aluminum alloy product may be hot formed after heating but before the rolled aluminum alloy product is quenched. The rolled aluminum alloy product as provided herein may have good ductility or formability at elevated temperatures. This may allow for the rolled aluminum alloy product to be malleable and achieve better formability. Hot forming the rolled aluminum alloy product when the product is at or near the first temperature may allow for the rolled aluminum alloy product to be formed into a variety of complex shapes. For example, after heating the rolled aluminum alloy product, the product may be transferred to a press or die where it is formed into a desired shape.

The rolled (and optionally formed) aluminum alloy product is quenched at block 1240. At block 1240, the rolled aluminum alloy product may be quenched to a second temperature of from about 10 °C to about 100 °C in a quenching process to generate a heat-treated aluminum alloy product. The second temperature may be ambient or room temperature in some embodiments. The quenching process may be performed using a slow quenching practice. The quenching rate in the slow quenching practice ranges from 0.5 °C per second to 125 °C per second. In some cases, the quenching rate may range from about 5 °C per second to about 125 °C per second.

In some embodiments, quenching the rolled aluminum alloy product at block 1240 may include two or more quenching processes. The rolled aluminum alloy product may be subjected to a first quenching to an intermediate temperature and then subjected to a second quenching until the rolled aluminum alloy product reaches the second temperature. For example, the rolled aluminum alloy product may be quenched from the first temperature to an intermediate temperature via a hot forming process. The intermediate temperature may be above the second temperature. Thus, a second quenching may be required to quench the rolled aluminum alloy product to the second temperature. The second quenching rate may be greater than the first quenching rate.

The heat-treated aluminum alloy product generated by the quenching process may exhibit superior mechanical properties over conventional aluminum alloy products. Specifically, the heat-treated aluminum alloy product as described herein exhibits a strain ratio of from 0.3 to 0.8. The strain ratio is determined according to an ASTM G129 standard test method. Other exemplary mechanical properties exhibited by the heat-treated aluminum alloy product may include an ultimate tensile strength of from 500 MPa to 650 MPa, a yield strength of from 400 MPa to 600 MPa, a uniform elongation of from 7.50% to 10.50%, and a total elongation of from 10.00% to 15.00%. The heat-treated aluminum alloy generated at block 1240 may be aluminum alloy products 210, 310, or aluminum alloy products 4A and 4B discussed with reference to FIG. 4, or aluminum alloy products 5A and 5B discussed with reference to FIGs. 5-11C. In some cases, the heat-treated aluminum alloy product may be a hot formed aluminum alloy product when the rolled aluminum alloy product is subjected to a hot forming process. In other cases, the heat-treated aluminum alloy product may be a formed aluminum alloy product when the rolled aluminum alloy product is subjected to one or more forming processes.

At block 1242, quenching the rolled aluminum alloy product may include subjecting the rolled aluminum alloy product to a water quenching process. Water quenching processes may include cold water immersion, hot water immersion, boiling water, or water spray. In various embodiments, quenching the rolled aluminum alloy product at block 1240 may include other methods of quenching. For example, block 1240 may include a forced air quenching process. Forced air quenching processes may include air blasts or still air procedures. Other quench methods that may be used at block 1240 may include polyalkylene glycol solutions, liquid nitrogen, fast quenching oils, or brine solutions.

Optionally, blocks 1230 and 1240 may be combined. For example, in some cases, the rolled aluminum alloy product may be quenched via a die quenching process. During a hot forming process, the rolled aluminum alloy product may be formed into parts using cold dies. Because the cold dies are cooler than the heated rolled aluminum alloy product, the cold dies may provide rapid quenching to the rolled aluminum alloy product. In some cases, the hot forming process may be considered to be part of the quenching process. In other cases, the rolled aluminum alloy product may be subjected to the hot forming process before or after the quenching process. In further cases, the hot forming process may occur between a first quenching process and a second quenching process.

After the rolled aluminum alloy product is quenched at block 1240, the heat-treated aluminum alloy product may be subjected to an aging process at block 1250. For example, the heat-treated aluminum alloy product may be subjected to a hardening process such as in a T6 or T7 temper. In some embodiments, the aging process at block 1250 may include re-heating the heat-treated aluminum alloy product to a temperature from about 100 °C to about 170 °C, maintaining the heat-treated aluminum alloy product at a temperature from about 100 °C to about 150 °C for a period of time, and cooling the sheet to a temperature near or at room temperature. In other cases, the aging process may include re-heating the heat-treated aluminum alloy product to a temperature from about 100 °C to about 150 °C; maintaining the heat-treated aluminum alloy product at a temperature from about 100 °C to about 150 °C for a period of time; heating the heat-treated aluminum alloy product to a temperature greater than about 150 °C; maintaining the heat-treated aluminum alloy product at a temperature greater than about 150 °C (e.g., from about 150 °C to about 170 °C) for a period of time; and cooling the heat-treated aluminum alloy product to room temperature. The heat-treated aluminum alloy product may be maintained at the temperature for a time period greater than 10 minutes, 20 minutes, 30 minutes, 40 minutes, 50 minutes, 60 minutes, 70 minutes, 80 minutes, 90 minutes, 100 minutes, 110 minutes, 2 hours, 6 hours, 12 hours, 18 hours, 24 hours, 30 hours, 32 hours, or 48 hours. For example, the heat-treated aluminum alloy product may be subjected to an aging process in which the product is re-heated to a temperature 100 °C to 170 °C and maintained at that temperature for 12 hours to 30 hours.

In some cases, the heat-treated aluminum alloy product may be subjected to paint bake heat treatment, for example, heating the heat-treated aluminum alloy product to a temperature greater than about 150 °C (e.g., 160 °C, 170 °C, 180 °C, 190 °C, 200 °C, or higher) and maintaining the heat-treated aluminum alloy product at the temperature greater than about 140 °C (e.g., between about 150 °C, 160 °C, 170 °C, 180 °C, 190 °C, 200 °C, or higher) for a period of time (e.g., 10 minutes, 20 minutes, 30 minutes, 40 minutes, 50 minutes, 60 minutes, 70 minutes, 80 minutes, 90 minutes, 100 minutes, 110 minutes, or 120 minutes).

Turning now to FIG. 13, graph 1300 illustrates a temperature profile of an aluminum alloy product as a function of time according to embodiments of the present disclosure. Graph 1300 may depict or correspond to an embodiment of a method of making a quench-insensitive aluminum alloy product. For example, graph 1300 may correspond to a method of making aluminum alloy product 210, 310, 4A, 4B, 5A, 5B, or any aluminum alloy product having a composition in accordance with Tables 1-6. Starting at step 1310, the rolled aluminum alloy product may be heated from room temperature to a first temperature of 480 °C during a heat treatment process. The heating may take approximately 50 seconds, as illustrated. In embodiments, room temperature may correspond to ambient conditions, such as approximately 40 °C. In this embodiment, the heat treatment process may be a solutionizing heat treatment process, indicated by the SHT notation. At step 1320, the rolled aluminum alloy product may be held at the first temperature for a time period, such as about 5 minutes. After this time period, the rolled aluminum alloy product may be quenched at step 1330 to generate a heat-treated aluminum alloy product. At step 1330, multiple quench rates are illustrated. For example, a quench rate of 550 °C/s, 350 °C/s, 150 °C/s, 50 °C/s, or 5 °C/s may be used at step 1330. Quenching at step 1330 may employ any of the various quenching methods discussed here. In some embodiments, the rolled aluminum alloy product may be quenched down to a second temperature, such as room temperature. Optionally, the heat-treated aluminum alloy product may be maintained at room temperature for 24 hours.

In some cases, the heat-treated aluminum alloy product may be subjected to an aging process. At step 1350, the heat-treated aluminum alloy product may be subjected to a T6 tempering process. Optionally, a T7 tempering process may be used. As provided on graph 1300, at step 1350 the heat-treated aluminum alloy product may be re-heated to a temperature of 125 °C. The heat-treated aluminum alloy product may be maintained at 125 °C for 24 hours before returning to room temperature.

### Methods of Using the Disclosed Aluminum Alloy Products

The aluminum alloy products described herein can be used in automotive applications and other transportation applications, including aircraft and railway applications. For example, the disclosed aluminum alloy products can be used to prepare automotive structural parts, such as bumpers, side beams, roof beams, cross beams, pillar reinforcements (e.g., A-pillars, B-pillars, and C-pillars), inner panels, outer panels, side panels, inner hoods, outer hoods, rockers, or trunk lid panels. The aluminum alloy products and methods described herein can also be used in aircraft or railway vehicle applications, to prepare, for example, external and internal panels. The aluminum alloy products described herein can be incorporated within upper wing, lower wing, or other body assemblies for aerospace applications.

The aluminum alloy products and methods described herein can also be used in electronics applications or any other desired application. For example, the aluminum alloy products and methods described herein can be used to prepare housings for electronic devices, including mobile phones and tablet computers. In some examples, the aluminum alloy products can be used to prepare housings for the outer casing of mobile phones (e.g., smart phones), tablet bottom chassis, and other portable electronics.

The foregoing description of the embodiments, including illustrated embodiments, has been presented only for the purpose of illustration and description and is not intended to be exhaustive or limiting to the precise forms disclosed. Numerous modifications, adaptations, and uses thereof will be apparent to those skilled in the art.

## Claims

1. A method comprising:
heating a rolled aluminum alloy product to a first temperature of from 400 °C to 525 °C wherein the rolled aluminum alloy product comprises a 7xxx series aluminum alloy comprising:
from 4.00 wt.% to 15.00 wt.% Zn,
from 0.30 wt.% to 2.50 wt.% Cu,
from 1.60 wt.% to 2.60 wt.% Mg,
from 0.10 wt.% to 0.25 wt.% Fe,
from 0.07 wt.% to 0.15 wt.% Si,
from 0.09 wt.% to 0.15 wt.% Zr,
from 0.02 wt.% to 0.05 wt.% Mn,
from 0.03 wt.% to 0.05 wt.% Cr,
from 0.003 wt.% to 0.035 wt.%Ti, and
remainder Al, with a maximum of 0.15 wt.% for the sum of all impurities, and wherein the rolled aluminum alloy product further comprises up to 0.20 wt.% of one or more of Mo, Nb, Be, B, Co, Sn, Sr, V, In, Hf, Ag, Sc and Ni; or
from 4.00 wt.% to 15.00 wt.% Zn,
from 0.20 wt.% to 2.10 wt.% Cu,
from 2.20 wt.% to 2.40 wt.% Mg,
from 0.18 wt.% to 0.23 wt.% Fe,
from 0.09 wt.% to 0.12 wt.% Si,
from 0.05 wt.% to 0.15 wt.% Zr,
from 0.04 wt.% to 0.09 wt.% Mn,
from 0.03 wt.% to 0.09 wt.% Cr,
from 0.01 wt.% to 0.02 wt.% Ti,
up to 0.15 wt.% of impurities, and
remainder Al, and wherein the rolled aluminum alloy product further comprises up to 0.20 wt.% of one or more of Mo, Nb, Be, B, Co, Sn, Sr, V, In, Hf, Ag, Sc and Ni;
maintaining the rolled aluminum alloy product at the first temperature or within 10 °C of the first temperature for a time duration of from 15 seconds to 30 minutes; and
quenching the rolled aluminum alloy product at a quench rate from 0.5 °C/s to 125 °C/s thereby generating a heat-treated aluminum alloy product, wherein the rolled aluminum alloy product is quenched until the rolled aluminum alloy product reaches a second temperature of from 10 °C to 100 °C, and wherein the heat-treated aluminum alloy product exhibits a strain ratio of from 0.3 to 0.8, and wherein the strain ratio is determined according to an ASTM G129 standard test method.

2. The method of claim 1, wherein quenching comprising a first quenching at a first quench rate to an intermediate temperature, a second quenching at a second quench rate to the second temperature, wherein the second quench rate is greater than the first quench rate; and/or
wherein the quench rate is from 5 °C/s to 125 °C/s; and/or
wherein the quench rate is from 10 °C/s to 125 °C/s.

3. The method of claim 1 or 2, wherein the first temperature is a solutionizing temperature; and/or
wherein the second temperature is ambient temperature; and/or
wherein heating and quenching the rolled aluminum alloy product correspond to a solutionizing heat treatment process; and/or
further comprising subjecting the rolled aluminum alloy product to a hot forming process after heating the rolled aluminum alloy product.

4. The method of any one of claims 1-3, wherein quenching the rolled aluminum alloy product comprises a die quenching process; and/or
wherein quenching the rolled aluminum alloy product comprises a water quenching process; and/or
wherein quenching the rolled aluminum alloy product comprises a forced air quenching process.

5. The method of any one of claims 1-4, further comprising aging the heat-treated aluminum alloy product to a T6 temper; and/or
further comprising aging the heat-treated aluminum alloy product to a T7 temper; and/or
further comprising heating the heat-treated aluminum alloy product to a temperature from 100 °C to 170 °C and maintaining at the temperature for 12 hours to 30 hours.

## Patentansprüche

1. Verfahren, umfassend:
Erhitzen eines gewalzten Aluminiumlegierungsprodukts auf eine erste Temperatur von 400 °C bis 525 °C, wobei das gewalzte Aluminiumlegierungsprodukt eine Aluminiumlegierung der Serie 7xxx umfasst, umfassend:
von 4,00 Gew.-% bis 15,00 Gew.-% Zn,
von 0,30 Gew.-% bis 2,50 Gew.-% Cu,
von 1,60 Gew.-% bis 2,60 Gew.-% Mg,
von 0,10 Gew.-% bis 0,25 Gew.-% Fe,
von 0,07 Gew.-% bis 0,15 Gew.-% Si,
von 0,09 Gew.-% bis 0,15 Gew.-% Zr,
von 0,02 Gew.-% bis 0,05 Gew.-% Mn,
von 0,03 Gew.-% bis 0,05 Gew.-% Cr,
von 0,003 Gew.-% bis 0,035 Gew.-% Ti, und
Rest Al, mit einem Maximum von 0,15 Gew.-% für die Summe aller Verunreinigungen, und wobei das gewalzte Aluminiumlegierungsprodukt ferner bis zu
0,20 Gew.-% von einem oder mehreren von Mo, Nb, Be, B, Co, Sn, Sr, V, In, Hf, Ag, Sc und Ni umfasst; oder
von 4,00 Gew.-% bis 15,00 Gew.-% Zn,
von 0,20 Gew.-% bis 2,10 Gew.-% Cu,
von 2,20 Gew.-% bis 2,40 Gew.-% Mg,
von 0,18 Gew.-% bis 0,23 Gew.-% Fe,
von 0,09 Gew.-% bis 0,12 Gew.-% Si,
von 0,05 Gew.-% bis 0,15 Gew.-% Zr,
von 0,04 Gew.-% bis 0,09 Gew.-% Mn,
von 0,03 Gew.-% bis 0,09 Gew.-% Cr,
von 0,01 Gew.-% bis 0,02 Gew.-% Ti,
bis zu 0,15 Gew.-% Verunreinigungen und
Rest Al, und wobei das gewalzte Aluminiumlegierungsprodukt ferner bis zu 0,20 Gew.-% von einem oder mehreren von Mo, Nb, Be, B, Co, Sn, Sr, V, In, Hf, Ag, Sc und Ni umfasst;
Halten des gewalzten Aluminiumlegierungsprodukts bei der ersten Temperatur oder innerhalb von 10 °C der ersten Temperatur für eine Zeitdauer von 15 Sekunden bis 30 Minuten; und
Abschrecken des gewalzten Aluminiumlegierungsprodukts bei einer Abschreckrate von 0,5 °C/s bis 125 °C/s, wodurch ein hitzebehandeltes Aluminiumlegierungsprodukt erzeugt wird, wobei das gewalzte Aluminiumlegierungsprodukt abgeschreckt wird, bis das gewalzte Aluminiumlegierungsprodukt eine zweite Temperatur von 10 °C bis 100 °C erreicht, und wobei das hitzebehandelte Aluminiumlegierungsprodukt ein Dehnungsverhältnis von 0,3 bis 0,8 aufweist und wobei das Dehnungsverhältnis gemäß einem ASTM-G129-Standardtestverfahren bestimmt wird.

2. Verfahren nach Anspruch 1, wobei Abschrecken ein erstes Abschrecken bei einer ersten Abschreckrate auf eine Zwischentemperatur, ein zweites Abschrecken bei einer zweiten Abschreckrate auf die zweite Temperatur umfasst, wobei die zweite Abschreckrate größer als die erste Abschreckrate ist; und/oder
wobei die Abschreckrate von 5 °C/s bis 125 °C/s beträgt; und/oder
wobei die Abschreckrate von 10 °C/s bis 125 °C/s beträgt.

3. Verfahren nach Anspruch 1 oder 2, wobei die erste Temperatur eine Lösungsglühtemperatur ist; und/oder
wobei die zweite Temperatur Umgebungstemperatur ist; und/oder
wobei Erhitzen und Abschrecken des gewalzten Aluminiumlegierungsprodukts einem Lösungsglüh-Hitzebehandlungsprozess entsprechen; und/oder
ferner umfassend, Aussetzen des gewalzten Aluminiumlegierungsprodukts einem Warmformungsprozess nach Erhitzen des gewalzten Aluminiumlegierungsprodukts.

4. Verfahren nach einem der Ansprüche 1 bis 3, wobei Abschrecken des gewalzten Aluminiumlegierungsprodukts einen Pressformabschreckprozess umfasst; und/oder
wobei Abschrecken des gewalzten Aluminiumlegierungsprodukts einen Wasserabschreckprozess umfasst; und/oder
wobei Abschrecken des gewalzten Aluminiumlegierungsprodukts einen Gebläseluftabschreckprozess umfasst.

5. Verfahren nach einem der Ansprüche 1 bis 4, ferner umfassend Altern des hitzebehandelten Aluminiumlegierungsprodukts zu einem T6-Zustand; und/oder
ferner umfassend Altern des hitzebehandelten Aluminiumlegierungsprodukts zu einem T7-Zustand; und/oder
ferner umfassend Erhitzen des hitzebehandelten Aluminiumlegierungsprodukts auf eine Temperatur von 100 °C bis 170 °C und Halten bei der Temperatur für 12 Stunden bis 30 Stunden.

## Revendications

1. Procédé comprenant:
le chauffage d'un produit en alliage d'aluminium laminé à une première température de 400°C à 525°C, dans lequel le produit en alliage d'aluminium laminé comprend un alliage d'aluminium de la série 7xxx comprenant:
de 4,00 % en poids à 15,00 % en poids de Zn,
de 0,30 % en poids à 2,50 % en poids de Cu,
de 1,60 % en poids à 2,60 % en poids de Mg,
de 0,10 % en poids à 0,25 % en poids de Fe,
de 0,07 % en poids à 0,15 % en poids de Si,
de 0,09 % en poids à 0,15 % en poids de Zr,
de 0,02 % en poids à 0,05 % en poids de Mn,
de 0,03 % en poids à 0,05 % en poids de Cr,
de 0,003 % en poids à 0,035 % en poids de Ti, et
le reste Al, avec un maximum de 0,15 % en poids pour la somme de toutes les impuretés, et dans lequel le produit en alliage d'aluminium laminé comprend en outre jusqu'à 0,20 % en poids d'un ou plusieurs de Mo, Nb, Be, B, Co, Sn, Sr, V, In, Hf, Ag, Sc et Ni; ou
de 4,00 % en poids à 15,00 % en poids de Zn,
de 0,20 % en poids à 2,10 % en poids de Cu,
de 2,20 % en poids à 2,40 % en poids de Mg,
de 0,18 % en poids à 0,23 % en poids de Fe,
de 0,09 % en poids à 0,12 % en poids de Si,
de 0,05 % en poids à 0,15 % en poids de Zr,
de 0,04 % en poids à 0,09 % en poids de Mn,
de 0,03 % en poids à 0,09 % en poids de Cr,
de 0,01 % en poids à 0,02 % en poids de Ti,
jusqu'à 0,15 % en poids d'impuretés, et
le reste Al, et dans lequel le produit en alliage d'aluminium laminé comprend en outre jusqu'à 0,20 % en poids d'un ou plusieurs de Mo, Nb, Be, B, Co, Sn, Sr, V, In, Hf, Ag, Sc et Ni;
le maintien du produit en alliage d'aluminium laminé à la première température ou dans des limites de 10°C par rapport à la première température pendant une durée de 15 secondes à 30 minutes; et
la trempe du produit en alliage d'aluminium laminé à une vitesse de trempe de 0,5°C/s à 125°C/s, générant ainsi un produit en alliage d'aluminium traité thermiquement, dans lequel le produit en alliage d'aluminium laminé est trempé jusqu'à ce que le produit en alliage d'aluminium laminé atteigne une seconde température de 10°C à 100°C, et dans lequel le produit en alliage d'aluminium traité thermiquement présente un rapport de déformation de 0,3 à 0,8, et dans lequel le rapport de déformation est déterminé selon un procédé d'essai de la norme ASTM G129.

2. Procédé selon la revendication 1, dans lequel la trempe comprenant une première trempe à une première vitesse de trempe jusqu'à une température intermédiaire, une seconde trempe à une seconde vitesse de trempe jusqu'à la seconde température, dans lequel la seconde vitesse de trempe est supérieure à la première vitesse de trempe; et/ou
dans lequel la vitesse de trempe est de 5°C/s à 125°C/s; et/ou
dans lequel la vitesse de trempe est de 10°C/s à 125°C/s.

3. Procédé selon la revendication 1 ou 2, dans lequel la première température est une température de mise en solution; et/ou
dans lequel la seconde température est la température ambiante; et/ou
dans lequel le chauffage et la trempe du produit en alliage d'aluminium laminé correspondent à un processus de traitement thermique de mise en solution; et/ou
comprenant en outre la soumission du produit en alliage d'aluminium laminé à un processus de formage à chaud après le chauffage du produit en alliage d'aluminium laminé.

4. Procédé selon l'une quelconque des revendications 1 à 3, dans lequel la trempe du produit en alliage d'aluminium laminé comprend un processus de trempe en matrice; et/ou
dans lequel la trempe du produit en alliage d'aluminium laminé comprend un processus de trempe à l'eau; et/ou
dans lequel la trempe du produit en alliage d'aluminium laminé comprend un processus de trempe à l'air forcé.

5. Procédé selon l'une quelconque des revendications 1 à 4, comprenant en outre le vieillissement du produit en alliage d'aluminium traité thermiquement jusqu'à un état de traitement T6; et/ou
comprenant en outre le vieillissement du produit en alliage d'aluminium traité thermiquement jusqu'à un état de traitement T7; et/ou
comprenant en outre le chauffage du produit en alliage d'aluminium traité thermiquement jusqu'à une température de 100°C à 170°C et le maintien à cette température pendant 12 heures à 30 heures.
